

[54] LIGHT SENSITIVE SILVER HALIDE  
PHOTOGRAPHIC MATERIAL

[75] Inventors: **Masao Sasaki, Hadano; Toyoki Nishijima; Shun Takada**, both of Odawara; **Kaoru Onodera**, Sagamihara, all of Japan

[73] Assignee: **Konishiroku Photo Industry Co., Ltd.**, Tokyo, Japan

[21] Appl. No.: 275,647

[22] Filed: Nov. 23, 1988

## Related U.S. Application Data

[63] Continuation of Ser. No. 5,654, Jan. 21, 1987, abandoned.

## [30] Foreign Application Priority Data

Jan. 25, 1986 [JP] Japan ..... 61-14595

[51] Int. Cl. 5 ..... G03C 7/38  
[52] U.S. Cl. ..... 430/546; 430/551;  
430/558

[58] Field of Search ..... 430/551, 558, 386, 387,  
430/546

## [56] References Cited

## U.S. PATENT DOCUMENTS

|           |         |                       |         |
|-----------|---------|-----------------------|---------|
| 3,930,866 | 1/1976  | Oishi et al. ....     | 430/551 |
| 4,587,210 | 5/1986  | Ono et al. ....       | 430/551 |
| 4,588,679 | 5/1986  | Furutachi ....        | 430/558 |
| 4,632,617 | 11/1986 | Kaneko et al. ....    | 430/551 |
| 4,639,415 | 1/1987  | Kaneko et al. ....    | 430/551 |
| 4,675,275 | 6/1987  | Nishijima et al. .... | 430/372 |

## FOREIGN PATENT DOCUMENTS

0182486 5/1986 European Pat. Off. .

Primary Examiner—Paul R. Michl

Assistant Examiner—Mark R. Buscher

Attorney, Agent, or Firm—Finnegan, Henderson, Farabow, Garrett, and Dunner

## [57] ABSTRACT

A silver halide photographic material comprising a silver halide emulsion layer containing (1) a pyrazoloazole magenta coupler, (2) an anti-color-fading agent having an oxidation potential ( $E_{ox}$ ) of  $0.95(V) < E_{ox} < 1.50(V)$  and (3) a hydroquinone derivative.

13 Claims, No Drawings

## LIGHT SENSITIVE SILVER HALIDE PHOTOGRAPHIC MATERIAL

This application is a continuation of application Ser. No. 07/005,654, filed Jan. 21, 1987, now abandoned.

### FIELD OF THE INVENTION

This invention relates to a light-sensitive silver halide photographic material. More particularly, it relates to a light-sensitive silver halide photographic material having excellent color reproducibility and also remarkably improved in fastness to light of magenta dye images.

### BACKGROUND OF THE INVENTION

It has been well known that dye images are produced by subjecting a light-sensitive silver halide color photographic material (hereinafter "color photographic material") to imagewise exposure to effect color development, whereby an oxidized product of an aromatic primary amine type color developing agent couples with a coupler to form dyes including, for example, indophenol, indoaniline, indamine, azomethine, phenoxadine, phenadine and other dyes similar to these. In such a photographic system, generally employed is a color reproduction system utilizing the subtractive color process, in which used is a color photographic material comprising blue-sensitive, green-sensitive and red-sensitive silver halide emulsion layers containing couplers each having the relationship of complementary color, namely, couplers which color-develop in yellow, magenta and cyan, respectively.

The coupler used for formation of yellow color images includes, for example, acetoanilide type couplers, and, as the coupler for formation of magenta color images, for example, pyrazolone, pyrazolobenzimidazole, pyrazolotriazole or indazolone type couplers are known, and further, as the coupler for formation of cyan color images, for example, phenol or naphthol type couplers are generally used.

The dye images thus obtained are desired not to undergo any color change or color-fading even when exposed to light for a long period of time or preserved under the conditions of high temperature and high humidity. Also desired are those in which non-image portions of a color photographic material may not yellow by light, moisture or heat.

However, in the case of magenta couplers, yellow stain (or Y-stain) by light, at a non-image portion and color-fading by light, at a dye image portion are very largely caused as compared with those in the case of yellow couplers or cyan couplers, to often raise problems.

The coupler widely used for formation of magenta dye includes, for example, 1,2-pyrazol-5-on type couplers. It has been a serious problem that the magenta couplers of 1,2-pyrazol-5-on type have a secondary absorption at the vicinity of 430 nm in addition to a primary absorption at the vicinity of 550 nm, and therefore various studies have been made to solve such a problem.

A magenta coupler having an anilino group at the 3-position of the 1,2-pyrazol-5-on type coupler, which is small in the above-mentioned secondary absorption, is useful for obtaining, in particular, a color image for printing. This art is disclosed, for example, in U.S. Pat. No. 2,343,703, British Patent No. 1,059,994, etc.

However, the above magenta couplers have a disadvantage that they are extremely poor in the image stability, in particular, the fastness to light of dye images, to suffer from Y-stain at a non-image portion.

As a means for decreasing the secondary absorption at the vicinity of 430 nm of the above magenta coupler, there have been proposed magenta couplers including, for example, pyrazolobenzimidazoles disclosed in British Patent No. 1,047,612, indazolones disclosed in U.S. Pat. No. 3,770,447, and pyrazolotriazoles disclosed in U.S. Pat. No. 3,725,067, British Patent Nos. 1,252,418 and 1,334,515, Japanese Unexamined Patent Publications No. 162548/1984 and No. 171956/1984, etc. The dyes formed through these couplers shows extremely smaller secondary absorption at the vicinity of 430 nm than the dyes formed through the 1,2-pyrazol-5-on type coupler do, and thus, they are desirable from the viewpoint of the color reproducibility, and also they are advantageous in that they are desirably very little liable to generation of Y-stain at a non-image portion against light, heat and humidity.

However, in general, the azomethine dye to be formed through the magenta couplers of pyrazolotriazole type have very low fastness to light to seriously damage the performances of a color photographic material, in particular, a color photographic material for print, and therefore have not put into practical use in color photographic materials for print.

Japanese Unexamined Patent Publication also proposes a technique for improving the fastness to light of a magenta dye image obtained from 1H-pyrazolo-[3,2-C]-s-triazole type magenta coupler by using 1H-pyrazolo-[3,2-C]-s-triazole type magenta coupler in combination with a phenol type compound or a phenol ether type compound. However, even in the above technique, some are not only insufficient for preventing the color-fading of the above magenta dye image against light, but also accelerate the color-fading by light on the contrary.

In short, there has not been found any means for sufficiently improving the fastness to light when the above pyrazolotriazole type magenta couplers are used, and an improvement has been earnestly sought after.

### SUMMARY OF THE INVENTION

This invention has been made taking account of the above problems, and an object of this invention is to provide a light-sensitive silver halide photographic material having excellent color reproducibility, improved magenta dye image-fastness against light, and improved resistance against generation of color fog.

A second object of this invention is to provide a method of achieving great fastness to light in a magenta dye image excellent in the color reproducibility.

As a result of intensive studies, the present inventors have found that the above objects can be achieved by a light-sensitive silver halide photographic material having at least one silver halide emulsion layer on a support, wherein at least one layer of said silver halide emulsion layer contains a magenta coupler represented by General Formula (I) shown below and an anti-color-fading agent having an oxidation potential  $E_{ox}$  being  $0.95 \text{ (V)} \leq E_{ox} \leq 1.50 \text{ (V)}$ , and said layer further contains a hydroquinone derivative in an amount ranging between  $1 \times 10^{-3}$  and  $1 \times 10^{-1}$  per 1 mole of said magenta coupler.



General Formula (I)

wherein Z represents a group of nonmetal atoms necessary for formation of a nitrogen-containing heterocyclic ring; said ring formed by Z may have a substituent; X represents a hydrogen atom or a substituent eliminable through the reaction with an oxidized product of a color developing agent; and R represents a hydrogen atom or a substituent.

#### DETAILED DESCRIPTION OF THE INVENTION

This invention will be described below in detail.

In the magenta coupler according to this invention, represented by General Formula (I);



General Formula (I)

Z represents a group of nonmetal atoms necessary for formation of a nitrogen-containing heterocyclic ring; said ring formed by Z may have a substituent.

X represents a hydrogen atom or a substituent eliminable through the reaction with an oxidized product of a color developing agent.

And, R represents a hydrogen atom or a substituent.

The substituent represented by the above R may include, for example, a halogen atom, an alkyl group, a cycloalkyl group, an alkenyl group, a cycloalkenyl group, an alkynyl group, an aryl group, a heterocyclic group, an acyl group, a sulfonyl group, a sulfinyl group, a phosphonyl group, a carbamoyl group, a sulfamoyl group, a cyano group, a spiro compound residual group, a bridged hydrocarbon compound residual group, an alkoxy group, an aryloxy group, a heterocyclic oxy group, a siloxy group, an acyloxy group, a carbamoyloxy group, an amino group, an acylamino group, a sulfonamide group, an imide group, an ureido group, a sulfamoylamino group, an alkoxy carbonylamino group, an aryloxy carbonylamino group, an alkoxy carbonyl group, an aryloxy carbonyl group, an alkylthio group, an arylthio group and a heterocyclic thio group.

The halogen atom may include, for example, a chlorine atom and a bromine atom. Particularly preferred is a chlorine atom.

The alkyl group represented by R may preferably be those having 1 to 32 carbon atoms; the alkenyl group and the alkynyl group, each having 2 to 32 carbon atoms; the cycloalkyl group and the cycloalkenyl group, each having 3 to 12 carbon atoms, particularly 5 to 7 carbon atoms. The alkyl group, the alkenyl group and the alkynyl group each may be of straight chain structure or branched structure.

Also, these alkyl group, alkenyl group, alkynyl group, cycloalkyl group and cycloalkenyl group each may have a substituent including, for example, an aryl, a cyano, a halogen atom, a heterocyclic ring, a cycloalkyl, a cycloalkenyl, a spiro compound residual group, a bridged hydrocarbon compound residual group, and

besides these, those which are substituted through a carbonyl group such as an acyl, a carboxyl, a carbamoyl, an alkoxy carbonyl and an aryloxy carbonyl, and those which are substituted through a hetero atom

5 {specifically, those which are substituted through an oxygen atom such as a hydroxyl, an alkoxy, an aryloxy, a heterocyclic oxy, a siloxy, an acyloxy and a carbamoyloxy, those which are substituted through a nitrogen atom such as a nitro, an amino (including a dialkylamino, etc.), a sulfamoylamino, an alkoxy carbonylamino, an aryloxy carbonylamino, an acylamino, a sulfonamide, an imide and a ureido, those which are substituted through a sulfur atom such as an alkylthio, an arylthio, a heterocyclic thio, a sulfonyl, a sulfinyl and a sulfamoyl and those which are substituted through a phosphorus atom such as a phosphonyl, etc}.

More specifically, they include, for example, a methyl group, an ethyl group, an isopropyl group, a t-butyl group, a pentadecyl group, a heptadecyl group, 10 a 1-hexyl group, a 1,1'-dipentyl group, a 2-chloro-t-butyl group, a tri-fluoromethyl group, a 1-ethoxytridecyl group, a 1-methoxyisopropyl group, an ethyl methanesulfonyl group, a methyl 2,4-di-t-amylfenyo group, an anilino group, a 1-phenylisopropyl group, a 3-m-butanesulfonaminophenoxypropyl group, 15 a 3-4'-{ $\alpha$ -[4'-(p-hydroxybenzenesulfonyl)phenoxy]-dodecanoylamino}phenylpropyl group, a 3-{4'-[ $\alpha$ -(2'',4''-di-t-amylphenoxy)butanamide]phenyl}propyl group, a 4-[ $\alpha$ -(o-chlorophenoxy)tetradecanamido]phenoxypropyl group, an allyl group, a cyclopentyl group, a cyclohexyl group, etc.

The aryl group represented by R is preferably a phenyl group, and may have a substituent (for example, an alkyl group, an alkoxy group, an acylamino group, etc.).

More specifically, it may include a phenyl group, a 4-t-butylphenyl group, a 2,4-di-t-amylphenyl group, a 4-tetradecanamido phenyl group, a hexadicyloxyphenyl group, a 4'-[ $\alpha$ -(4''-t-butylphenoxy)tetradecanamido]phenyl group, etc.

The heterocyclic group represented by R is preferably one having 5- to 7-members, which may be substituted or condensed. More specifically, it may include a 2-furyl group, a 2-thienyl group, a 2-pyrimidinyl group, a 2-benzothiazolyl group, etc.

The acyl group represented by R may include, for example, alkylcarbonyl groups such as an acetyl group, a phenyl acetyl group, a dodecanoyl group and an  $\alpha$ -2,4-di-t-amylphenoxybutanoyl group; arylcarbonyl groups such as a benzoyl group, a 3-pentadecyloxybenzoyl group and a p-chlorobenzoyl group; etc.

The sulfonyl group represented by R may include alkylsulfonyl groups such as a methylsulfonyl group and a dodecylsulfonyl group; arylsulfonyl groups such as a benzenesulfonyl group and a p-toluenesulfonyl group; etc.

The sulfinyl group represented by R may include alkylsulfinyl groups such as an ethylsulfinyl group, an octylsulfinyl group and a 3-phenoxybutylsulfinyl group; arylsulfinyl groups such as a phenylsulfinyl group, a m-pentadecylphenylsulfinyl group; etc.

The phosphonyl group represented by R may include alkylsulfonyl groups such as a butyloctylphosphonyl group, alkoxyphosphonyl groups such as an octyloxyphosphonyl group, aryloxyphosphonyl groups such as a phenoxyphosphonyl group, arylphosphonyl groups such as a phenylphosphonyl group, etc.

The carbamoyl group represented by R may be substituted with an alkyl group, an aryl group (preferably, a phenyl group), etc., and may include, for example, an N-methylcarbamoyl group, an N,N-dibutylcarbamoyl group, an N-(ethyl 2-pentadecyloctyl)carbamoyl group, an N-ethyl-N-dodecylcarbamoyl group, an N-[3-(2,4-di-t-amylphenoxy)propyl]carbamoyl group, etc.

The sulfamoyl group represented by R may be substituted with an alkyl group, an aryl group (preferably a phenyl group), etc., and may include, for example, an N-propylsulfamoyl group, an N,N-diethylsulfamoyl group, an N-(2-pentadecyloxyethyl)sulfamoyl group, an N-ethyl-N-dodecylsulfamoyl group, an N-phenylsulfamoyl group, etc.

The spiro compound residual group represented by R 15 may include, for example, spiro[3.3]heptan-1-yl, etc.

The bridged hydrocarbon compound residual group may include, for example, bicyclo[2.2.1]heptan-1-yl, tricyclo[3.3.1.1<sup>3,7</sup>]decan-1-yl, 7,7-dimethyl-dibicyclo[2.2.1]heptan-1-yl, etc.

The alkoxy group represented by R may be further substituted with those mentioned as the substituents for the above alkyl group, and may include, for example, a methoxy group, a propoxy group, a 2-ethoxyethoxy group, a pentadecyloxy group, a 2-dodecyloxyethoxy 25 group, a phenethoxyethoxy group, etc.

The aryloxy group represented by R is preferably a phenoxy, wherein the aryl nucleus may be further substituted with those mentioned as the substituents for the above aryl group, and may include, for example, a 30 phenoxy group, a p-t-butylphenoxy group, a m-pentadecylphenoxy group, etc.

The heterocyclic oxy group represented by R is preferably one having 5- to 7-members, wherein the heterocyclic ring may further have a substituent, and may 35 include, for example, a 3,4,5,6-tetrahydropyranyl-2-oxy group, a 1-phenyltetrazole-5-oxy group, etc.

The siloxy group represented by R may further be substituted with an alkyl group, etc., and may include, for example, a trimethylsiloxy group, a triethylsiloxy 40 group, a dimethylbutylsiloxy group, etc.

The acyloxy group represented by R may include, for example, an alkylcarbonyloxy group, an arylcarbonyloxy group, etc., and may further have a substituent to include, specifically, an acetoxy group, an  $\alpha$ -45 chloroacetoxy group, a benzoxyloxy group, etc.

The carbamoyloxy group represented by R may be substituted with an alkyl group, an aryl group, etc., and may include, for example, an N-ethylcarbamoyloxy group, an N,N-diethylcarbamoyloxy group, an N-phenylcarbamoyloxy group, etc.

The amino group represented by R may be substituted with an alkyl group, an aryl group (preferably, a phenyl group), and may include, for example, an ethylamino group, an anilino group, a m-chloroanilino 55 group, a 3-pentadecyloxycarbonylanilino group, a 2-chloro-5-hexadecanamidoanilino group, etc.

The acylamino group represented by R may include an alkylcarbonylamino group, an arylcarbonylamino group (preferably, a phenylcarbonylamino group), etc., and may further have a substituent to include, specifically, an acetoamide group, an  $\alpha$ -ethylpropaneamide group, an N-phenylacetamide group, a dodecanamide group, a 2,4-di-t-amylphenoxyacetamide group, an  $\alpha$ -3-t-butyl-4-hydroxyphenoxybutaneamide group, etc.

The sulfonamide group represented by R may include an alkylsulfonylamino group, an arylsulfonylamino group, and may further have a substituent. It specifici-

cally may include, a methylsulfonylamino group, a pentadecylsulfonylamino group, a benzenesulfonamide group, a p-toluenesulfonamide, a 2-methoxy-5-t-amylbenzenesulfonamide group, etc.

The imide group represented by R may be of open chain structure or cyclic structure, or may have a substituent to include, for example, a succinimide group, a 3-heptadecylsuccinimide, a phthalimide group, a glutalimide group, etc.

The ureido group represented by R may be substituted with an alkyl group, an aryl group (preferably, a phenyl group), etc., and may include, for example, an N-ethylureido group, an N-ethyl-N-decylureido group, an N-phenylureido group, an N-p-tolylureido group, etc.

The sulfamoylamino group represented by R may be substituted with an alkyl group or an aryl group (preferably, a phenyl group), etc., and may include, for example, an N,N-dibutylsulfamoylamino group, an N-methylsulfamoylamino group, an N-phenylsulfamoylamino group, etc.

The alkoxy carbonylamino group represented by R may further have a substituent, and may include, for example, a methoxycarbonylamino group, a methoxyethoxycarbonylamino group, an octadecyloxycarbonylamino group, etc.

The aryloxycarbonylamino group represented by R may have a substituent, and may include, for example, a phenoxy carbonylamino group, a 4-methylphenoxy carbonylamino group, etc.

The alkoxy carbonyl group represented by R may further have a substituent, and may include, for example, a methoxycarbonyl group, a butyloxycarbonyl group, a dodecyloxycarbonyl group, an octadecyloxycarbonyl group, an ethoxymethoxycarbonyloxy group, a benzyloxycarbonyl group, etc.

The aryloxycarbonyl group represented by R may further have a substituent, and may include, for example, a phenoxy carbonyl group, a p-chlorophenoxy carbonyl group, an m-pentadecyloxyphenoxy carbonyl group, etc.

The alkylthio group represented by R may further have a substituent, and may include, for example, an ethylthio group, a dodecylthio group, an octadecylthio group, a phenethylthio group, a 3-phenoxypropylthio group, etc.

The arylthio group represented by R is preferably a phenylthio group which may further have a substituent, and may include, for example, a phenylthio group, a p-methoxyphenylthio group, a 2-t-octylphenylthio group, a 3-octadecylphenylthio group, a 2-carboxyphenylthio group, a p-acetoaminophenylthio group, etc.

The heterocyclic thio group represented by R is preferably a heterocyclic thio group of 5 to 7 members, and may further have a condensed ring or may have a substituent. It may include, for example, a 2-pyridylthio group, a 2-benzothiazolylthio group, a 2,4-diphenoxy-1,3,5-triazole-6-thio group, etc.

The substituent represented by X, which is eliminable through the reaction with an oxidized product of a color developing agent, may include, for example, a halogen atom (such as a chlorine atom, a bromine atom and a fluorine atom), and also groups which are substituted through a carbon atom, an oxygen atom, a sulfur atom or a nitrogen atom.

The groups which are substituted through a carbon atom may include a carboxyl group, and also, for example, a group represented by the general formula:



wherein R' is same as defined for the above R, Z' is same as defined for the above Z; and R<sup>2</sup>' and R<sup>3</sup>' each represent a hydrogen atom, an aryl group, an alkyl group or a heterocyclic group, a hydroxymethyl group and a triphenylmethyl group.

The groups which are substituted through an oxygen atom may include, for example, an alkoxy group, aryloxy group, heterocyclic oxy group, an acyloxy group, a sulfonyloxy group, an alkoxy carbonyloxy group, an aryloxycarbonyloxy group, an alkyloxycarbonyloxy group, an alkoxyxaryloxy group, an alkoxyxaryloxy group, etc.

The above alkoxy group may further have a substituent including, for example, an ethoxy group, a 2-phenoxyethoxy group, 2-cyanoethoxy group, a phenoxy group, a p-chlorobenzoyloxy group, etc.

The above aryloxy group is preferably a phenoxy group, and the aryl group may further have a substituent. More specifically, it may include a phenoxy group, a 3-methylphenoxy group, a 3-dodecylphenoxy group, a 4-methanesulfonamidephenoxy group, a 4-[ $\alpha$ -(3'-pentadecylphenoxy)butanamido]phenoxy group, a hexadecylcarbamoylmethoxy group, a 4-cyanophenoxy group, a 4-methanesulfonylphenoxy group, a 1-naphthoxy group, a p-methoxyphenoxy group, etc.

The above heterocyclic oxy group is preferably a heterocyclic oxy group of 5 to 7 members, or may be of condensed ring, or may have a substituent. Specifically, it may include a 1-phenyltetrazolyl group, a 2-benzothiazolyl group, etc.

The above acyloxy group may include, for example, alkylcarbonyloxy groups such as an acetoxy group and butanoloxy group, and alkenylcarbonyloxy groups such as a cinnamoyloxy group, and arylcarbonyloxy groups such as a benzoyloxy group.

The above sulfonyloxy group may include, for example, a butanesulfonyloxy group and methanesulfonyloxy group.

The above alkoxy carbonyloxy group may include, for example, an ethoxycarbonyloxy group and a benzoyloxycarbonyloxy group.

The above aryloxycarbonyloxy group may include a phenoxy carbonyloxy group, etc.

The above alkyloxycarbonyloxy group may include, for example, a methyloxycarbonyloxy group.

The above alkoxyoxalyl group may include an ethoxyoxalyl group, etc.

The group which is substituted through a sulfur atom may include, for example, an alkylthio group, an arylthio group, a heterocyclic thio group and an alkyloxythiocarbonylthio group.

The above alkylthio group may include a butylthio group, a 2-cyanoethylthio group, a phenethylthio group, a benzylthio group, etc.

The above arylthio group may include a phenylthio group, a 4-methanesulfonamidephenylthio group, a 4-dodecylphenethylthio group, a 4-nonafluoropen-tanamidephenethylthio group, a 4-carboxyphenylthio group, a 2-ethoxy-5-t-butylphenylthio group, etc.

The above heterocyclic thio group may include, for example, a 1-phenyl-1,2,3,4-tetrazolyl-5-thio group, a 2-benzothiazolylthio group, etc.

The above alkyloxythiocarbonylthio group may include a dodecyloxythiocarbonylthio group, etc.

The group which is substituted through a nitrogen atom may include, for example, a group represented by the general formula:



In this formula, R<sup>4</sup>' and R<sup>5</sup>' each represent a hydrogen atom, an alkyl group, an aryl group, a heterocyclic group, a sulfamoyl group, a carbamoyl group, an acyl group, a sulfonyl group, an aryloxycarbonyl group or an alkoxy carbonyl group, and R<sup>4</sup>' and R<sup>5</sup>' may be bonded to each other to form a heterocyclic ring, provided that R<sup>4</sup>' and R<sup>5</sup>' each are not a hydrogen atom at the same time.

The above alkyl group may be of straight chain or branched one, and is preferably one having 1 to 22 carbon atoms. Also, this alkyl group may have a substituent which may include, for example, an aryl group, an alkoxy group, an aryloxy group, an alkylthio group, an arylthio group, an alkylamino group, arylamino group, an acylamino group, a sulfonamide group, an imino group, an acyl group, an alkylsulfonyl group, an arylsulfonyl group, a carbamoyl group, a sulfamoyl group, an alkoxy carbonyl group, an alkyloxycarbonylamino group, an aryloxycarbonylamino group, a hydroxyl group, a carboxyl group, a cyano group and a halogen atom. The alkyl group may specifically include, for example, an ethyl group, an octyl group, a 2-ethylhexyl group and 2-chloroethyl group.

The aryl group represented by R<sup>4</sup>' or R<sup>5</sup>' is preferably one having 6 to 32 carbon atoms, in particular, a phenyl group and a naphthyl group, wherein the aryl group may have a substituent which may include those mentioned as the substituents for the alkyl group represented by the above R<sup>4</sup>' or R<sup>5</sup>'. This aryl group may specifically include, for example, a phenyl group, a 1-naphthyl group and a 4-methylsulfonylphenyl group.

The heterocyclic group represented by R<sup>4</sup>' or R<sup>5</sup>' is preferably of 5 to 6 members, or may be of condensed ring, or may have a substituent. Specifically, it may include a 2-furyl group, a 2-quinolyl group, a 2-pyrimidyl group, a 2-benzothiazolyl group, a 2-pyridyl group, etc.

The sulfamoyl group represented by R<sup>4</sup>' or R<sup>5</sup>' may include an N-alkylsulfamoyl group, an N,N-dialkylsulfamoyl group, N-arylsulfamoyl group, an N,N-diaryl-sulfamoyl group, etc., and the alkyl group and the aryl group of these may have the substituent mentioned for the above alkyl group and aryl group. The sulfamoyl group may specifically include, for example, an N,N-diehtylsulfamoyl group, an N-methylsulfamoyl group, N-dodecylsulfamoyl group and an N-p-tolylsulfamoyl group.

The carbamoyl group represented by R<sup>4</sup>' or R<sup>5</sup>' may include an N-alkylcarbamoyl group, an N,N-dialkylcarbamoyl group, an N-arylcaramoyl group, an N,N-diarylcarbamoyl group, etc., and the alkyl group and the aryl group of these may have the substituent mentioned for the above alkyl group and aryl group. The

carbamoyl group may specifically include, for example, an N,N-diethylcarbamoyl group, an N-methylcarbamoyl group, an N-dodecylcarbamoyl group, N-p-cyano-phenylcarbamoyl group and N-p-tolylcarbamoyl group.

The acyl group represented by R<sup>4</sup> or R<sup>5</sup> may include, for example, an alkylcarbonyl group, an arylcarbonyl group and a heterocyclic carbonyl group, and the alkyl group, the aryl group and the heterocyclic group each may have a substituent. The acyl group may specifically include, for example, a hexafluorobutanoyl group, 2,3,4,5,6-pentafluorobenzoyl group, an acetyl group, a benzoyl group, a naphthoel group, a 2-furylcarbonyl group, etc.

The sulfonyl group represented by R<sup>4</sup> or R<sup>5</sup> may include an alkylsulfonyl group, an arylsulfonyl group and a heterocyclic sulfonyl group, and may have a substituent. Specifically, it may include, for example, an ethanesulfonyl group, a benzenesulfonyl group, an octanesulfonyl group, a naphthalenesulfonyl group, a p-chlorobenzenesulfonyl group, etc.

The aryloxycarbonyl group represented by R<sup>4</sup> or R<sup>5</sup> may have as a substituent those mentioned for the above aryl group. Specifically, it may include a phenoxy carbonyl group, etc.

The alkoxy carbonyl group represented by R<sup>4</sup> or R<sup>5</sup> may have the substituent mentioned for the above alkyl group, and specifically may include a methoxycarbonyl group, a dodecyloxycarbonyl group, a benzyloxycarbonyl group, etc.

The heterocyclic ring to be formed by bonding of R<sup>4</sup> and R<sup>5</sup> is preferably of 5 to 6 members, and may be saturated or unsaturated, may be aromatic or non-aromatic, or may be of a condensed ring. This heterocyclic ring may include, for example, an N-phthalimide group, an N-succinimide group, a 4-N-urazolyl group, a 1-N-hydantoinyl group, 3-N-2,4-dioxoazazolyl group, a 2-N-1,1-dioxo-3-(2H)-oxo-1,2-benzthiazolyl group, a 1-pyrol group, a 1-pyrolidinyl group, a 1-pyrazolyl group, a 1-pyrazolylidinyl group, a 1-piperidinyl group, a 1-pyrolinyl group, a 1-imidazolyl group, a 1-imidazolinyl group, a 1-indolyl group, 1-isindolinyl group, a 2-isindolyl group, a 2-isindolinyl group, a 1-benzotriazolyl group, a 1-benzimidazolyl group, a 45 1-(1,2,4-triazolyl) group, a 1-(1,2,3-triazolyl) group, a 1-(1,2,3,4-tetrazolyl) group, an N-morpholinyl group, a 1,2,3,4-tetrahydroquinolyl group, a 2-oxo-1-pyrrolidinyl group, a 2-1H-pyrrolidone group, a phthaladione group, a 2-oxo-1-piperidinyl group, etc., and these heterocyclic groups each may be substituted with an alkyl group, an aryl group, an alkoxy group, an aryloxy group, an acyl group, a sulfonyl group, an alkylamino group, an arylamino group, an acylamino group, a sulfonamino group, a carbamoyl group, a sulfamoyl group, an alkylthio group, an arylthio group, a ureido group, an alkoxy carbonyl group, an aryloxycarbonyl group, an imide group, a nitro group, a cyano group, a carboxyl group, a halogen atom, etc.

The nitrogen-containing heterocyclic ring to be formed by Z or Z' may include a pyrazole ring, an imidazole ring, a triazole ring, a tetrazole ring, etc., and the substituent which the above rings each may have include those mentioned for the above R.

When the substituents (for example, R, R<sup>1</sup> to R<sup>6</sup>) on 65 the heterocyclic rings in General Formula (I) and General Formulas (II) to (VIII) shown hereinbelow have a moiety of:



wherein R'', X and Z'' each have the same meaning as

R, X, and Z in General Formula (I),

a so-called bis-body type coupler is formed, which may be included in this invention as a matter of course. Also, on the rings formed by Z, Z', Z'' and the later-mentioned Z<sup>1</sup>, other rings (for example, a cycloalkene of 5 to 7 members) may be further condensed. For instance, in General Formula (V), R<sup>5</sup> and R<sup>6</sup> may be, and, in General Formula (VI), R<sup>7</sup> and R<sup>8</sup> may be bonded to each other to form a ring (for example, a 5- to 7-membered cycloalkene, benzene).

The coupler represented by General Formula (I) may, more specifically, be represented, for example, by General Formulas (II) to (VII) shown below:



General Formula (II)



General Formula (III)



General Formula (IV)



General Formula (V)



General Formula (VI)



General Formula (VII)



General Formula (VIII)

In the above General Formulas (II) to (VII), R<sup>1</sup> to R<sup>8</sup> and X each have the same meaning as R and X mentioned before.

Also, what is most preferable in General Formula (I) is one represented by General Formula (VIII) shown below:

wherein  $R^1$ ,  $X$  and  $Z^1$  each have the same meaning as  $R$ ,  $X$  and  $Z$  in General Formula (I).

Of the magenta couplers represented by the above General Formulas (II) to (VII), particularly preferred is the magenta coupler represented by General Formula (II).

As for the substituents on the heterocyclic rings in General Formula (I) to (VIII), it is preferable for  $R$ , in the case of General Formula (I), and for  $R^1$ , in the cases of General Formulas (II) to (VIII), to each satisfy the condition 1 shown below, and it is further preferable to satisfy the conditions 1 and 2 shown below, and it is particularly preferable to satisfy the conditions 1, 2 and 3 shown below:

Condition 1: A root atom directly bonded to the heterocyclic ring is a carbon atom.

Condition 2: Only one hydrogen atom is bonded to the above carbon atom, or not bonded thereto at all.

Condition 3: All of the bonds between the carbon atom and atoms adjoining thereto are in single bonding.

Substituents most preferable as the substituents  $R$  and  $R^1$  in the above heterocyclic rings include those represented by General Formula (IX) shown below:



General Formula (IX)

In the above formula,  $R^9$ ,  $R^{10}$  and  $R^{11}$  each represent a hydrogen atom, a halogen atom, an alkyl group, a cycloalkyl group, an alkenyl group, a cycloalkenyl group, an alkynyl group, an aryl group, a heterocyclic group, an acyl group, a sulfonyl group, a sulfinyl group, a phosphonyl group, a carbamoyl group, a sulfamoyl group, a cyano group, a spiro compound residual group, a bridged hydrocarbon compound residual group, an alkoxy group, an aryloxy group, a heterocyclic oxy group, a siloxy group, an acyloxy group, a carbamoyloxy group, an amino group, an acylamino group, a sulfonamide group, an imide group, a ureido group, a sulfamoyl amino group, an alkoxy carbonyl amino group, an aryloxycarbonyl amino group, an alkoxy carbonyl group, an aryloxycarbonyl group, an alkylthio group, an arylthio group, a heterocyclic thio group; and at least two of  $R^9$ ,  $R^{10}$  and  $R^{11}$  are not hydrogen atoms.

Two substituents in the above  $R^9$ ,  $R^{10}$  and  $R^{11}$ , for example,  $R^9$  and  $R^{10}$ , may be bonded to form a saturated or unsaturated ring (for example, a cycloalkane, a cycloalkene, a heterocyclic ring), or  $R^{11}$  may be further bonded to this ring to form a residue of a bridged hydrocarbon compound.

The groups represented by  $R^9$  to  $R^{11}$  may have a substituent, and examples of the groups represented by  $R^9$  to  $R^{11}$  and the substituents these groups may have, may include the specific examples and the substituents mentioned for the group represented by  $R$  in General Formula (I).

Also, examples of the ring to be formed by bonding, for instance, of  $R^9$  and  $R^{10}$  and the residue of bridged hydrocarbon compound to be formed by  $R^9$  to  $R^{11}$ , and also the substituents which this ring may have, may include the specific examples and the substituents mentioned for the cycloalkyl, the cycloalkenyl and the residue of heterocyclic bridged hydrocarbon compound

which are represented by  $R$  in the above General Formula (I).

In General Formula (X), preferable are;

(i) the case where two of  $R^9$  to  $R^{11}$  are each an alkyl group; and

(ii) the case where one of  $R^9$  to  $R^{11}$ , for example,  $R^{11}$  is a hydrogen atom, and the other two,  $R^9$  and  $R^{10}$  are bonded to form a cycloalkyl together with the carbon atoms at the root.

Further preferable in the case (i) is the case where two of  $R^9$  to  $R^{11}$  are each an alkyl group, and the other one is a hydrogen atom or an alkyl group.

Here, the alkyl and the cycloalkyl each may further have a substituent, and examples of the alkyl, the cycloalkyl and the substituents of these may include those for the alkyl, the cycloalkyl and the substituents of these which are represented by  $R$  in the above General Formula (I).

The substituents which the ring to be formed by  $Z$  in General Formula (I) and the ring to be formed by  $Z^1$  in General Formula (VIII) may have, and the substituents  $R^2$  to  $R^8$  in General Formulas (II) to (VI), are preferably those represented by General Formula (X) shown below:



General Formula (X)

wherein  $R^1$  represents an alkylene group,  $R^2$  represents an alkyl group, a cycloalkyl group or an aryl group.

The alkylene represented by  $R^1$  preferably has 2 or more, and more preferably 3 to 6 carbon atoms at the straight chain portion, and may be of straight chain or branched structure. Also, this alkylene may have a substituent.

Examples of such substituent may include those shown as the substituents which the alkyl group when  $R$  in General Formula (I) may have.

Preferable substituents may include a phenyl. Preferable examples for the alkylene represented by  $R^1$  are shown below:



The alkyl group represented by  $R^2$  may be of straight chain or branched structure. Specifically, it may include methyl, ethyl, propyl, iso-propyl, butyl, 2-ethylhexyl, octyl, dodecyl, tetradecyl, hexadecyl, octadecyl, 2-hexyldecyl, etc.

The cycloalkyl group represented by  $R^2$  is preferably of 5 to 6 members, and may include, for example, a cyclohexyl group.

The alkyl group and the cycloalkyl group represented by  $R^2$  may each have a substituent including, for

example, those exemplified as the substituents for the above R<sup>1</sup>.

The aryl group represented by R<sup>2</sup> may specifically include a phenyl group and a naphthyl group. The aryl group may have a substituent. Such a substituent may include, for example, a straight chain or branched alkyl group, and besides, those exemplified as the substituents for the above R<sup>1</sup>.

Also, when there are two or more substituents, they may be the same or different substituents.

Particularly preferable in the compounds represented by General Formula (I) are those represented by General Formula (XI) shown below:

General Formula (XI)



wherein R and X each have the same meaning as R and X in General Formula (I), and R<sup>1</sup> and R<sup>2</sup> each have the same meaning as R<sup>1</sup> and R<sup>2</sup> in General Formula (X).

Specific examples of the compounds used in this invention are shown below:



-continued



8



9



10



11



12



13



14



15



16

-continued



17



18



19



20



21



22



23



24

-continued



25



26



27



28



29



30



31



32



33

-continued



-continued



40



41



42



43



44



45



46



47



48

-continued



49



50



51



52



53



54



55



56



57

-continued



-continued



-continued



75



76



77



78



79



80



81



82



83

-continued



84



85



86



87



88



89



90



9

-continued

92



93



94



95



96



97



98



99





-continued



101



102



103



104



105



106



107



108

-continued



109



110



111



112



113



114



115

-continued

116



117



118



119



120



121



122



123

-continued

124



125



126



127



128



129



130



131



-continued

132



133



134



135



136



137



138



139



-continued

140



141



142



143



144



145



146



147



-continued

148



149



150



151



152



153



154



155



156



-continued



157



158



159



160



161



162



163



164



165



166

-continued



-continued



173



174



175



176



177



178



179

-continued



180



181



182



183



184



185



186



187

-continued



188



189



190



191



192



193



194



195

-continued



196



197



198



199



200



201



202



203



204

-continued



205



206



207



208



209



210



211



212

-continued



213



214



215



216



217



218



219



220



-continued



Syntheses of the above couplers can be carried out by making reference to Journal of the Chemical Society, Perkin I, 1977, pp 2047-2052, U.S. Pat. No. 3,725,067 and Japanese Unexamined Patent Publication Nos. 99437/1984, 42045/1983, 162548/1984, 171956/1984, 33552/1985, 43659/1985, 172982/1985 and 190779/1985, etc.

The couplers of this invention can be used usually in the range of  $1 \times 10^{-3}$  mole to 1 mole, preferably  $1 \times 10^{-2}$  to  $8 \times 10^{-1}$  mole, per 1 mole of silver halide.

The couplers of this invention can be also used in combination with magenta couplers of other kinds.

The hydroquinone derivative used in this invention and described below in detail, which is the compound known as a stain preventive agent, have been conventionally known to have an effect as an anti-color-fading agent of a magenta dye formed from a magenta coupler for photography, as disclosed in Japanese Unexamined Patent Publication Nos. 24141/1983 and 180557/1984.

However, as a result of various studies, the present inventors found that high fastness to light can not be achieved in respect of only the magenta dye formed from the magenta coupler represented by the above General Formula (I), so long as the above hydroquinone derivative is used in an amount in which it is usually used conventionally as the anti-color-fading agent, and, as a result of further studies, they discovered that a greatest effect can be obtained only when the above hydroquinone derivative is used in a particular amount, by using together an anti-color-fading agent having an oxidation potential  $E_{ox}$  being  $0.95 (V) \leq E_{ox} \leq 1.50 (V)$ .

The anti-color-fading agent, used in this invention, having an oxidation potential  $E_{ox}$  being  $0.95 (V) \leq E_{ox} \leq 1.50 (V)$  (hereinafter called "anti-color-fading agent according to this invention) will be described below in detail.

The oxidation potential  $E_{ox}$  of the anti-color-fading agent according to this invention can be readily measured by a person skilled in the art. Methods for the measurement are disclosed, for example, in papers by A. Stanienda, "Naturwissenschaften" Vol. 47, pages 353 and 512 (1960); P. Delahay, "New Instrumental Methods in Electrochemistry" (1954) published by Interscience Publishers; L. Meites, "Polarographic Tech-

niques", 2nd Ed. (1965), published by Interscience Publishers; etc.

The above  $E_{ox}$  value refers to the potential at which an electron of the compound is withdrawn at an anode in voltammetry, and primarily relates to the highest occupied electron energy level in the ground state of the compound.

The  $E_{ox}$  in this invention is a value obtained from the half-wave potential of a polarograph under the conditions shown below. That is, the value was measured by using acetonitrile as a solvent for the anti-color-fading agent, and 0.1N sodium perchlorate as a supporting electrolyte, setting the density of the anti-color-fading agent to  $10^{-3}$  to  $10^{-4}$  mole/lit., using an Ag/AgCl electrode as a reference electrode, using a rotated platinum plate electrode for the measurement of  $E_{ox}$ , and at 25° C.

So far as the anti-color-fading agent according to this invention has the oxidation potential being in the range mentioned above, the compounds of any structure can be used. In particular, however, preferable compounds may include those represented by General Formulas (A) to (H), (J) and (K) shown below, and more preferably the compounds represented by General Formulas (A), (B), (G) and (J). As a matter of course, even the compounds other than those represented by these General Formulas may be used as the anti-color-fading agent according to this invention if they have the oxidation potential in the range mentioned above.

General Formula (A)



In the formula,  $R^1$  represents a hydrogen atom, an alkyl group, an alkenyl group, an aryl group or a heterocyclic group;  $R^2$ ,  $R^3$ ,  $R^5$  and  $R^6$  each represent a hydrogen atom, a halogen atom, a hydroxyl group, an alkyl group, an alkenyl group, an ary group, an alkoxy group or an acylamino group;  $R^4$  represents an alkyl

group, a hydroxyl group, an aryl group or an alkoxy group, provided that when  $R^1$  is a hydrogen atom,  $R^4$  is other than a hydroxyl group.  $R^1$  and  $R^2$  may be combined with each other to form a 5- or 6-membered ring, whereas  $R^4$  represents a hydroxyl group or an alkoxy group. Also,  $R^3$  and  $R^4$  may be combined to form a hydrocarbon ring of 5 members, whereas  $R^1$  represents an alkyl group, an aryl group or a heterocyclic group.

In the above General Formula (A), wherein  $R^1$  represents a hydrogen atom, an alkyl group, an alkenyl group, an aryl group or a heterocyclic group, the alkyl group may include, for example, straight-chain or branched alkyl groups such as a methyl group, an ethyl group, a propyl group, n-octyl group, tert-octyl group and hexadecyl group. The alkenyl group represented by  $R^1$  may include, for example, an allyl group, a hexenyl group, an octenyl group, etc. Further, the aryl group represented by  $R^1$  may include each of a phenyl group and a naphthyl group. Further, the heterocyclic group represented by  $R^1$  may include, specifically, a tetrahydropyranyl group, a pyrimidyl group, etc. These groups may each have a substituent. For example, as the alkyl group having a substituent, it may include a benzyl group and an ethoxymethyl group; as the aryl group having a substituent, a methoxyphenyl group, a chlorophenyl group, a 4-hydroxy-3,5-dibutylphenyl group, etc.

In General Formula (A), wherein  $R^2$ ,  $R^3$ ,  $R^5$  and  $R^6$  each represent a hydrogen atom, a halogen atom, a hydroxyl group, an alkyl group, an alkenyl group, an aryl group, an alkoxy group or an acylamino group, the alkyl group, the alkenyl group and the aryl group may include the alkyl group, the alkenyl group and the aryl group mentioned for the above  $R^1$ . Also, the above halogen atom may include, for example, fluorine, chlorine, bromine, etc. Further, the above alkoxy group may include specifically a methoxy group, an ethoxy group, etc. Further, the above acylamino group is represented by  $R'CONH-$ , wherein  $R'$  represents an alkyl group (for example, groups such as methyl, ethyl, n-propyl, n-butyl, n-octyl, tert-octyl and benzyl), an alkenyl group (for example, groups such as allyl, octinyl and oleyl), an aryl group (for example, groups such as phenyl, methoxyphenyl and naphthyl) or a heterocyclic group (for example, groups such as pyridyl and pyrimidyl).

In the above General Formula (A), wherein  $R^4$  represents an alkyl group, a hydroxyl group, an aryl group or an alkoxy group, the alkyl group and the aryl group may include specifically those same as in the alkyl group and the aryl group represented by the above  $R^1$ . Also, the alkoxy group represented by  $R^4$  may include those same as in the alkoxy group mentioned for the above  $R^2$ ,  $R^3$ ,  $R^5$  and  $R^6$ .

The ring formed together with a benzene by ring closure of  $R^1$  and  $R^2$  may include, for example, chroman, coumaran and methylenedioxybenzene. Also, the ring formed together with a benzene ring by ring closure of  $R^3$  and  $R^4$  may include, for example, indane. These rings may have a substituent (for example, alkyl, alkoxy and aryl).

An atom in the ring formed by ring closure of  $R^1$  and  $R^2$  or ring closure of  $R^3$  and  $R^4$  may be a spiro atom to form a spiro compound, or  $R^2$  and  $R^4$  may be a linking group to form a bis-type compound.

Of the phenol type compounds and the phenylether type compounds represented by the above General Formula (A), preferable is a biindane compound having

four  $RO-$  groups (wherein  $R$  represents an alkyl group, an alkenyl group, an aryl group or a heterocyclic group), particularly preferable is a compound represented by General Formula (A-1) shown below:



In the formula,  $R$  represents an alkyl group (for example, methyl, ethyl, propyl, n-octyl, tert-octyl, benzyl and hexadecyl), an alkenyl group (for example, allyl, octenyl and oleyl), an aryl group (for example, phenyl and naphthyl) or a heterocyclic group (for example, tetrahydropyranyl and pyrimidyl).  $R^9$  and  $R^{10}$  each represent a hydrogen atom, a halogen atom (for example, fluorine, chlorine and bromine), an alkyl group (for example, methyl, ethyl, n-butyl and benzyl), an allyl group (for example, allyl, hexenyl and octenyl) or an alkoxy group (for example, methoxy, ethoxy and benzyloxy);  $R^{11}$  represents a hydrogen atom, an alkyl group (for example, methyl, ethyl, n-butyl and benzyl), an alkenyl group (for example, 2-propenyl, hexenyl and octenyl) or an aryl group (for example, phenyl, methoxyphenyl, chlorophenyl and naphthyl).

The compound represented by the above General Formula (A) may also include the compounds disclosed in U.S. Pat. Nos. 3,935,016, 3,982,944 and 4,254,216, Japanese Unexamined Patent Publication Nos. 21004/1980 and 145530/1979, British Patent Publication Nos. 2,077,455 and 2,062,888, U.S. Pat. Nos. 3,764,337, 3,432,300, 3,574,627 and 3,573,050, Japanese Unexamined Patent Publication Nos. 152225/1977, 20327/1978, 17729/1978 and 6321/1980, British Patent No. 1,347,556, British Patent Publication No. 2,066,975, Japanese Patent Publication Nos. 12337/1979 and 31625/1973, U.S. Pat. No. 3,700,455, etc.



In the formula,  $R^1$  and  $R^4$  each represents a hydrogen atom, a halogen atom, an alkyl group, an alkenyl group, an alkoxy group, an alkenyloxy group, a hydroxy group, an aryl group, an aryloxy group, an acyl group, an acylamino group, an acyloxy group, a sulfonamide group, a cycloalkyl group, or an alkoxy carbonyl group;  $R^2$  represents a hydrogen atom, an alkyl group, an alkenyl group, an aryl group, an acyl group, a cycloalkyl group or a heterocyclic group; and  $R_3$  represents a hydrogen atom, a halogen atom, an alkyl group, an alkenyl group, an aryl group, an aryloxy group, an acyl group, an acyloxy group, a sulfonamide group, a cycloalkyl group or an alkoxy carbonyl group.

The above-mentioned groups each may be substituted with other substituent which may include, for example, an alkyl group, an alkenyl group, an alkoxy

group, an aryl group, an aryloxy group, a hydroxyl group, an alkoxy carbonyl group, an aryloxycarbonyl group, an acylamino group, an acyloxy group, a carbamoyl group, a sulfonamide group, a sulfamoyl group, etc.

Also,  $R^2$  and  $R^3$  may be combined each other to form a 5- or 6-membered ring. The ring formed together with a benzene ring by the ring closure of  $R^2$  and  $R^3$  may include, for example, a chroman ring and a methyleneoxybenzene ring.

$Y$  represents a group of atoms necessary for formation of a chroman or coumaran ring.

The chroman or coumaran ring may be substituted with a halogen atom, an alkyl group, a cycloalkyl group, an alkoxy group, an alkenyl group, an alkenyloxy group, a hydroxyl group, an aryl group, an aryloxy group or a heterocyclic group, or may further form a spiro ring.

Of the compounds represented by General Formula (B), compounds most useful for this invention are included in the compounds represented by General Formulas (B-1), (B-2), (B-3), (B-4) and (B-5).



$R^1$ ,  $R^2$ ,  $R^3$  and  $R^4$  in General Formulas (B-1), (B-2), (B-3), (B-4) and (B-5) have the same meaning as those in the above General Formula (B), and  $R^5$ ,  $R^6$ ,  $R^7$ ,  $R^8$ ,  $R^9$  and  $R^{10}$  each represents a hydrogen atom, a halogen atom, an alkyl group, an alkoxy group, a hydroxyl

group, an alkenyl group, an alkenyloxy group, an aryl group, an aryloxy group or a heterocyclic group.

Also,  $R^5$  and  $R^6$ ,  $R^6$  and  $R^7$ ,  $R^7$  and  $R^8$ ,  $R^8$  and  $R^9$ , and  $R^9$  and  $R^{10}$  each may be cyclized each other to form a carbon ring, and such a carbon ring may be further substituted with an alkyl group.

In the above General Formulas (B-1), (B-2), (B-3), (B-4) and (B-5), particularly useful compounds are those in which  $R^1$  and  $R^4$  are each a hydrogen atom, an alkyl group, an alkoxy group, a hydroxyl group or a cycloalkyl group, and  $R^5$ ,  $R^6$ ,  $R^7$ ,  $R^8$ ,  $R^9$  and  $R^{10}$  are each a hydrogen atom, an alkyl group or a cycloalkyl group.

The compounds represented by General Formula (B) include the compounds disclosed in Tetrahedron Letters, 1970, Vol. 126, pp 4743-4751; Japan Chemical Society, 1972, No. 10, pp 0987-1990; Chem. Lett., 1972, (4), pp 315-316 and Japanese Unexamined Patent Publication No. 139383/1980, and may be synthesized by the methods also disclosed in these publications.



In the above formulas,  $R^1$  and  $R^2$  each represent a hydrogen atom, a halogen atom, an alkyl group, an alkenyl group, an alkoxy group, an alkenyloxy group, a hydroxyl group, an aryl group, an aryloxy group, an acyl group, an acylamino group, an acyloxy group, a sulfonamide group or an alkoxy carbonyl group.

The groups mentioned above each may be substituted with other substituent which may include, for example, a halogen atom, an alkyl group, an alkenyl group, an alkoxy group, an aryloxy group, a hydroxyl group, an alkoxy carbonyl group, an aryloxycarbonyl group, an acylamino group, a carbamoyl group, a sulfonamide group, a sulfamoyl group, etc.

$Y$  represents a group of atoms necessary for formation of a dichroman or dicoumaran ring together with a benzene ring.

Chroman or coumaran ring may be substituted with a halogen atom, an alkyl group, a cycloalkyl group, an alkoxy group, an alkenyl group, alkenyloxy group, a hydroxyl group, an aryl group, an aryloxy group or a heterocyclic group, or further may form a spiro ring.

Of the compounds represented by General Formulas (C) and (D), compounds most useful for this invention are included in the compounds represented by General Formulas (C-1), (C-2), (D-1) and (D-2), respectively.



and (D-2) have the same meaning as those in General Formulas (C) and (D), and R<sup>3</sup>, R<sup>4</sup>, R<sup>5</sup>, R<sup>6</sup>, R<sup>7</sup> and R<sup>8</sup> each represent a hydrogen atom, a halogen atom, an alkyl group, an alkoxy group, a hydroxyl group, an alkenyl group, an alkenyloxy group, an aryl group, an aryloxy group or a heterocyclic ring. Also, R<sup>3</sup> and R<sup>4</sup>, R<sup>4</sup> and R<sup>5</sup>, R<sup>5</sup> and R<sup>6</sup>, R<sup>6</sup> and R<sup>7</sup> and R<sup>7</sup> and R<sup>8</sup> each may be cyclized each other to form a carbon ring, and such a carbon ring may be further substituted with alkyl group.

In the above General Formulas (C-1), (C-2), (D-1) and (D-2), particularly useful compounds are those in which R<sup>1</sup> and R<sup>2</sup> are each a hydrogen atom, an alkyl group, an alkoxy group, a hydroxyl group or a cycloalkyl group, and R<sup>3</sup>, R<sup>4</sup>, R<sup>5</sup>, R<sup>6</sup>, R<sup>7</sup> and R<sup>8</sup> are each a hydrogen atom, an alkyl group or a cycloalkyl group.

The compounds represented by General Formulas (C) and (D) include the compounds disclosed in Japan Chemical Society, Part C, 1968. (14), p 1937-18; Organic Synthetic Chemical Association, 1970, 28(1), pp 60-65; Tetrahedron Letters, 1973. (29), pp 2707-2710, and may be synthesized by the methods also disclosed in these publications.



General Formula (C-1)

5 In the formula, R<sup>1</sup> represents a hydrogen atom, an alkyl group, an alkenyl group, an aryl group, an acyl group, a cycloalkyl group or a heterocyclic group; and R<sup>3</sup> represents a hydrogen atom, a halogen atom, an alkyl group, an alkenyl group, an aryl group, an aryloxy group, an acyl group, an acylamino group, an acyloxy group, a sulfonamide group, a cycloalkyl group or an alkoxy carbonyl group.

General Formula (C-2)

10 R<sup>2</sup> and R<sup>4</sup> each represents a hydrogen atom, a halogen atom, an alkyl group, an alkenyl group, an aryl group, an acyl group, an acylamino group, a sulfonamide group, a cycloalkyl group or an alkoxy carbonyl group.

15 The above-mentioned groups each may be substituted with other substituent which may include, for example, an alkyl group, an alkenyl group, an alkoxy group, an aryl group, an aryloxy group, a hydroxyl group, an alkoxy carbonyl group, an aryloxycarbonyl group, an acylamino group, a carbamoyl group, a sulfonamide group, a sulfamoyl group, etc.

20 Also, R<sup>1</sup> and R<sup>2</sup> may be combined each other to form a 5- or 6-membered ring.

25 In that occasion, R<sup>3</sup> and R<sup>4</sup> each represents a hydrogen atom, a halogen atom, an alkyl group, an alkenyl group, an alkoxy group, an alkenyloxy group, a hydroxyl group, an aryl group, an aryloxy group, an acyl group, an acylamino group, an acyloxy group, a sulfonamide group or an alkoxy carbonyl group.

30 Y represents a group of atoms necessary for formation of a chroman or coumaran ring.

35 The chroman or coumaran ring may be substituted with a halogen atom, an alkyl group, a cycloalkyl group, an alkoxy group, an alkenyl group, an alkenyloxy group, a hydroxyl group, an aryl group, an aryloxy group or a heterocyclic group, or may further form a spiro ring.

40 Of the compounds represented by General Formula (E), compounds most useful for this invention are included in the compounds represented by General Formulas (E-1), (E-2), (E-3), (E-4) and (E-5).



General Formula (E)



In the formula, R<sup>1</sup> represents a hydrogen atom, an alkyl group, an alkenyl group, an aryl group, an acyl group, a cycloalkyl group or a heterocyclic group; and R<sup>3</sup> represents a hydrogen atom, a halogen atom, an alkyl group, an alkenyl group, an aryl group, an aryloxy group, an acyl group, an acylamino group, an acyloxy group, a sulfonamide group, a cycloalkyl group or an alkoxy carbonyl group.

R<sup>2</sup> and R<sup>4</sup> each represents a hydrogen atom, a halogen atom, an alkyl group, an alkenyl group, an aryl group, an acyl group, an acylamino group, a sulfonamide group, a cycloalkyl group or an alkoxy carbonyl group.

The above-mentioned groups each may be substituted with other substituent which may include, for example, an alkyl group, an alkenyl group, an alkoxy group, an aryl group, an aryloxy group, a hydroxyl group, an alkoxy carbonyl group, an aryloxycarbonyl group, an acylamino group, a carbamoyl group, a sulfonamide group, a sulfamoyl group, etc.

Also, R<sup>1</sup> and R<sup>2</sup> may be combined each other to form a 5- or 6-membered ring.

In that occasion, R<sup>3</sup> and R<sup>4</sup> each represents a hydrogen atom, a halogen atom, an alkyl group, an alkenyl group, an alkoxy group, an alkenyloxy group, a hydroxyl group, an aryl group, an aryloxy group, an acyl group, an acylamino group, an acyloxy group, a sulfonamide group or an alkoxy carbonyl group.

Y represents a group of atoms necessary for formation of a chroman or coumaran ring.

The chroman or coumaran ring may be substituted with a halogen atom, an alkyl group, a cycloalkyl group, an alkoxy group, an alkenyl group, an alkenyloxy group, a hydroxyl group, an aryl group, an aryloxy group or a heterocyclic group, or may further form a spiro ring.

Of the compounds represented by General Formula (E), compounds most useful for this invention are included in the compounds represented by General Formulas (E-1), (E-2), (E-3), (E-4) and (E-5).

75



$R^1$ ,  $R^2$ ,  $R^3$  and  $R^4$  in Formulas (E-1) to (E-5) have the same meaning as those in the above Formula (E), and  $R^5$ ,  $R^6$ ,  $R^7$ ,  $R^8$ ,  $R^9$  and  $R^{10}$  each represents a hydrogen atom, a halogen atom, an alkyl group, an alkoxy group, a hydroxyl group, an alkenyl group, an alkenyloxy group, an aryl group, an aryloxy group or a heterocyclic group.

Further,  $R^5$  and  $R^6$ ,  $R^6$  and  $R^7$ ,  $R^7$  and  $R^8$ ,  $R^8$  and  $R^9$ , and  $R^9$  and  $R^{10}$  each may be cyclized with each other to form a carbon ring, and such a carbon ring may be further substituted with an alkyl group. . . .

In the above Formulas (E-1) to (E-5), particularly useful compounds are those in which  $R^1$ ,  $R^2$ ,  $R^3$  and  $R^4$  are each a hydrogen atom, an alkyl group or a cycloalkyl group; and in the above Formula (E-5),  $R^3$  and  $R^4$  are each a hydrogen atom, an alkyl group, an alkoxy group, a hydroxyl group or a cycloalkyl group; and in the above Formulas (E-1) to (E-5),  $R^5$ ,  $R^6$ ,  $R^7$ ,  $R^8$ ,  $R^9$  and  $R^{10}$  are each a hydrogen atom, an alkyl group or a cycloalkyl group. 40

The compounds represented by Formula (E) include the compounds disclosed in *Tetrahedron Letters*, 1965, (8), pp 457-460; *Japan Chemical Society, Part C*, 1966, (22), pp 2013-2016; *Zh. Org. Khim.*, 1970, (6), pp 45 1230-1237, and may be synthesized by the methods also disclosed in these publications.



In the formula,  $R^1$  represents a hydrogen atom, an alkyl group, an alkenyl group, an acyl group, a cycloalkyl group or a heterocyclic group;  $R^2$  represents a hydrogen atom, a halogen atom, an alkyl group, an alkenyl group, an aryl group, aryloxy group, an acyl group, an acylamino group, an acyloxy group, a sulfonamide group, a cycloalkyl group or an alkoxy carbonyl group.

$R^3$  represents a hydrogen atom, a halogen atom, an 65 alkyl group, an alkenyl group, an aryl group, an acyl group, an acylamino group, a sulfonamide group, a cycloalkyl group or an alkoxy carbonyl group.

76

$R^4$  represents a hydrogen atom, a halogen atom, an alkyl group, an alkenyl group, an alkoxy group, an alkenyloxy group, a hydroxyl group, an aryl group, an aryloxy group, an acyl group, an acylamino group, an acyloxy group, a sulfonamide group or an alkoxy carbonyl group.

The above-mentioned groups each may be substituted with other substituent which may include, for example, an alkyl group, an alkenyl group, an alkoxy group, an aryl group, an aryloxy group, a hydroxyl group, an alkoxy carbonyl group, an aryloxy carbonyl group, an acylamino group, a carbamoyl group, a sulfonamide group, a sulfamoyl group, etc.

Also,  $R^1$  and  $R^2$  may be combined each other to form 15 a 5- or 6-membered ring. In this occasion,  $R^3$  and  $R^4$  each represents a hydrogen atom, a halogen atom, an alkyl group, an alkenyl group, an alkoxy group, an alkenyloxy group, a hydroxyl group, an aryl group, an aryloxy group, an acyl group, an acylamino group, an 20 acyloxy group, a sulfonamide group or an alkoxy carbonyl group.

Y represents a group of atoms necessary for formation of a chroman or coumaran ring.

25 The chroman or coumaran ring may be substituted with a halogen atom, an alkyl group, a cycloalkyl group, an alkoxy group, an alkenyl group, an alkenyloxy group, a hydroxyl group, an aryl group, an aryloxy group or a heterocyclic group, or may further form a spiro ring.

30 Of the compounds represented by General Formula (F), compounds most useful for this invention are included in the compounds represented by General Formulas (F-1), (F-2), (F-3), (F-4) and (F-5).



-continued



General Formula (F-5)

$R^1$ ,  $R^2$ ,  $R^3$  and  $R^4$  in General Formulas (F-1) to (F-5) have the same meaning as those in the above General Formula (F), and  $R^5$ ,  $R^6$ ,  $R^7$ ,  $R^8$ ,  $R^9$  and  $R^{10}$  each represent a hydrogen atom, a halogen atom, an alkyl group, an alkoxy group, a hydroxyl group, an alkenyl group, an alkenyloxy group, an aryl group, an aryloxy group or a heterocyclic group.

Further,  $R^5$  and  $R^6$ ,  $R^6$  and  $R^7$ ,  $R^7$  and  $R^8$ ,  $R^8$  and  $R^9$ , and  $R^9$  and  $R^{10}$  each may be cyclized each other to form a carbon ring, and such a carbon ring may be further substituted with an alkyl group.

Also, in General Formulas (F-3), (F-4) and (F-5),  $R^1$  to  $R^{10}$  in two of them each may be the same or different.

In the above General Formulas (F-1), (F-2), (F-3), (F-4) and (F-5), particularly useful compounds are those in which  $R^1$ ,  $R^2$  and  $R^3$  are each a hydrogen atom, an alkyl group or a cycloalkyl group;  $R^4$  is a hydrogen atom, an alkyl group, an alkoxy group, a hydroxyl group or a cycloalkyl group; and further,  $R^5$ ,  $R^6$ ,  $R^7$ ,  $R^8$ ,  $R^9$  and  $R^{10}$  are each a hydrogen atom, an alkyl group or a cycloalkyl group.

The compounds represented by General Formula (F) include the compounds disclosed in Tetrahedron Letters, 1970, Vol. 26, pp 4743-4751; Japan Chemical Society, 1972, No. 10, pp 1987-1990; Synthesis, 1975, Vol. 6, pp 392-393; and Bul. Soc. Chim. Belg., 1975, Vol. 84(7), pp 747-759, and may be synthesized by the methods disclosed in these publications.



General Formula (G)

In the formula,  $R^1$  and  $R^3$  each represent a hydrogen atom, a halogen atom, an alkyl group, an alkenyl group, an alkoxy group, a hydroxyl group, an aryl group, an aryloxy group, an acyl group, an acylamino group, an acyloxy group, a sulfonamide group, a cycloalkyl group or an alkoxy carbonyl group.

$R^2$  represents a hydrogen atom, a halogen atom, an alkyl group, an alkenyl group, a hydroxyl group, an aryl group, an acyl group, an acylamino group, an acyloxy group, a sulfonamide group, a cycloalkyl group or an alkoxy carbonyl group.

The above-mentioned groups each may be substituted with other substituent which may include, for example, an alkyl group, an alkenyl group, an alkoxy group, an aryl group, an aryloxy group, a hydroxyl group, an alkoxy carbonyl group, an aryloxy carbonyl group, an acylamino group, a carbamoyl group, a sulfonamide group, a sulfamoyl group, etc.

Also,  $R^2$  and  $R^3$  may be combined each other to form a 5- or 6-membered hydrocarbon ring. This 5- or 6-membered hydrocarbon ring may be substituted with a

halogen atom, an alkyl group, a cycloalkyl group, an alkoxy group, an alkenyl group, a hydroxyl group, an aryl group, an aryloxy group or a heterocyclic group.

5  $Y$  represents a group of atoms necessary for formation of an indane ring. The indane ring may be substituted with a halogen atom, an alkyl group, an alkenyl group, an alkoxy group, a cycloalkyl group, a hydroxyl group, an aryl group, an aryloxy group or a heterocyclic group, or may further form a spiro ring.

10 Of the compounds represented by General Formula (G), compounds most useful for this invention are included in the compounds represented by General Formulas (G-1) to (G-3).



General Formula (G-1)



General Formula (G-2)



General Formula (G-3)

$R^1$ ,  $R^2$  and  $R^3$  in General Formulas (G-1) to (G-3) have the same meaning as those in the above General Formula (G), and  $R^4$ ,  $R^5$ ,  $R^6$ ,  $R^7$ ,  $R^8$  and  $R^9$  each represent a hydrogen atom, an alkyl group, an alkoxy group, an alkenyl group, a hydroxyl group, an aryl group, an aryloxy group or a heterocyclic group.  $R^4$  and  $R^5$ ,  $R^5$  and  $R^6$ ,  $R^6$  and  $R^7$ ,  $R^7$  and  $R^8$ , and  $R^8$  and  $R^9$  each may be combined each other to form a hydrocarbon ring, and such a hydrocarbon ring may be further substituted with an alkyl group.

60 In the above General Formulas (G-1) to (G-3), particularly useful compounds are those in which  $R^1$  and  $R^3$  are each a hydrogen atom, an alkyl group, an alkoxy group, a hydroxyl group or a cycloalkyl group;  $R^2$  is a hydrogen atom, an alkyl group, a hydroxyl group or a cycloalkyl group; and  $R^4$ ,  $R^5$ ,  $R^6$ ,  $R^7$ ,  $R^8$  and  $R^9$  are each a hydrogen atom, an alkyl group or a cycloalkyl group.



General Formula (H)

In the formula, R<sup>1</sup> and R<sup>2</sup> each represent a hydrogen atom, a halogen atom, an alkyl group, an alkenyl group, an aryl group, an acyl group, an acylamino group, an acyloxy group, a sulfonamide group, a cycloalkyl group or an alkoxy carbonyl group.

R<sup>3</sup> represents a hydrogen atom, a halogen atom, an alkyl group, an alkenyl group, an alkoxy group, a hydroxyl group, an aryl group, an aryloxy group, an acyl group, an acylamino group, an acyloxy group, a sulfonamide group, a cycloalkyl group or an alkoxy carbonyl group.

The above-mentioned groups each may be substituted with other substituent which may include, for example, an alkyl group, an alkenyl group, an alkoxy group, an aryl group, an aryloxy group, a hydroxyl group, an alkoxy carbonyl group, an aryloxy carbonyl group, an acylamino group, a carbamoyl group, a sulfonamide group, a sulfamoyl group, etc.

Also, R<sup>1</sup> and R<sup>2</sup>, and R<sup>2</sup> and R<sup>3</sup> each may be combined each other to form a 5- or 6-membered hydrocarbon ring, and the hydrocarbon ring may be substituted with a halogen atom, an alkyl group, a cycloalkyl group, an alkoxy group, an alkenyl group, a hydroxyl group, an aryl group, an aryloxy group or a heterocyclic group.

Y represents a group of atoms necessary for formation of an indane ring. The indane ring may be substituted with a group capable of substituting the above hydrocarbon ring, or may further form a spiro ring.

Of the compounds represented by General Formula (H), compounds most useful for this invention are included in the compounds represented by General Formulas (H-1) to (H-3).



General Formula (H-1)



General Formula (H-2)

-continued



General Formula (H-3)

R<sup>1</sup>, R<sup>2</sup> and R<sup>3</sup> in General Formulas (H-1) to (H-3) have the same meaning as those in the above General Formula (H), and R<sup>4</sup>, R<sup>5</sup>, R<sup>6</sup>, R<sup>7</sup>, R<sup>8</sup> and R<sup>9</sup> each represents a hydrogen atom, a halogen atom, an alkyl group, an alkoxy group, a hydroxyl group, an alkenyl group, an aryl group, an aryloxy group or a heterocyclic group. R<sup>4</sup> and R<sup>5</sup>, R<sup>5</sup> and R<sup>6</sup>, R<sup>6</sup> and R<sup>7</sup>, R<sup>7</sup> and R<sup>8</sup>, and R<sup>8</sup> and R<sup>9</sup> each may be ring-closed each other to form a hydrocarbon ring, and such a hydrocarbon ring may be further substituted with an alkyl group.

In the above General Formulas (H-1) to (H-3), particularly useful compounds are those in which R<sup>1</sup> and R<sup>2</sup> are each a hydrogen atom, an alkyl group or a cycloalkyl group; R<sup>3</sup> is a hydrogen atom, an alkyl group, an alkoxy group, a hydroxyl group or a cycloalkyl group; and R<sup>4</sup>, R<sup>5</sup>, R<sup>6</sup>, R<sup>7</sup>, R<sup>8</sup> and R<sup>9</sup> are each a hydrogen atom, an alkyl group or a cycloalkyl group.

Synthesis method of the above compounds represented by General Formula (H) is known, and they may be synthesized in accordance with U.S. Pat. No. 3,057,929; Chem. Bar., 1972, 95(5), pp 1673-1674; Chemistry Letters, 1980, pp 739-742.

General Formula (J)



40 In the formula, R<sup>1</sup> represents an aliphatic group, a cycloalkyl group or an aryl group; and Y represents a group of nonmetal atoms necessary for forming a heterocyclic ring of 5 to 7 members together with a nitrogen atom; provided that, when two or more hetero atoms are present in the nonmetal atom containing a nitrogen atom for forming the heterocyclic ring, at least two hetero atoms are hetero atoms which are not contiguous to each other.

45 The aliphatic group represented by R<sup>1</sup> may include a saturated alkyl group which may have a substituent and an unsaturated alkyl group which may have a substituent. The saturated alkyl group may include, for example, a methyl group, an ethyl group, a butyl group, an octyl group, a dodecyl group, a tetradecyl group, a hexadecyl group, etc., and the unsaturated alkyl group may include, for example, ethenyl group, a propenyl group, etc.

50 The cycloalkyl group represented by R<sup>1</sup> may include a 5- to 7-membered cycloalkyl group which may have a substituent, which may include, for example, a cyclopentyl group, a cyclohexyl group, etc.

55 The aryl group represented by R<sup>1</sup> may include a phenyl group and a naphthyl group, which respectively may have a substituent.

60 The substituents for the aliphatic group, the cycloalkyl group and the aryl group represented by R<sup>1</sup> may include an alkyl group, an aryl group, an alkoxy group, a carbonyl group, a carbamoyl group, an acylamino

group, a sulfamoyl group, a sulfonamide group, a carbonyloxy group, an alkylsulfonyl group, an arylsulfonyl group, a hydroxyl group, a heterocyclic group, an alkylthio group, an arylthio group, etc., and these substituents may further have a substituent.

In the above General Formula (J), Y, which represents a group of nonmetal atoms necessary for forming a heterocyclic ring of 5 to 7 members together with a nitrogen atom, at least two of the nonmetal atoms containing a nitrogen atom for forming the heterocyclic ring must be hetero atoms, and this at least two hetero atoms must not be contiguous to each other. If, in the heterocyclic ring of the compound represented by General Formula (J), all of the hetero atoms are contiguous to each other, the performance as a magenta dye image stabilizing agent will not be attained, undesirably.

The above heterocyclic ring of 5 to 7 members of the compound represented by General Formula (J) may have a substituent, and the substituent may include an alkyl group, an aryl group, an acyl group, a carbamoyl group, an alkoxy carbonyl group, a sulfonyl group, a sulfamoyl group, etc., which may further have a substituent. Also, the heterocyclic ring of 5 to 7 members may be saturated, and a saturated heterocyclic ring is preferred. Further, a benzene ring, etc. may be condensed, or a spiro ring may be formed.

Of the compounds represented by General Formula (J), particularly preferable are piperazine type compounds and homopiperazine type compounds, and more preferably, they are the compounds represented by General Formula (J-1) or (J-2) shown below:

General Formula (J-1)



General Formula (J-2)



In the formulas, R<sup>2</sup> and R<sup>3</sup> each represent a hydrogen atom, an alkyl group or an aryl group, provided that R<sup>2</sup> and R<sup>3</sup> are not hydrogen atoms at the same time. R<sup>4</sup> to R<sup>13</sup> each represent a hydrogen atom, an alkyl group or an aryl group.

In the above General Formulas (J-1) and (J-2) wherein R<sup>2</sup> and R<sup>3</sup> each represent a hydrogen atom, an alkyl group or an aryl group, the alkyl group represented by R<sup>2</sup> or R<sup>3</sup> may include, for example, a methyl group, an ethyl group, a butyl group, an octyl group, a dodecyl group, a tetradecyl group, a hexadecyl group, an octadecyl group, etc. The aryl group represented by R<sup>2</sup> or R<sup>3</sup> may include a phenyl group, etc. The alkyl group and the aryl group represented by R<sup>2</sup> or R<sup>3</sup> may have a substituent, and the substituent may include a halogen atom, an alkyl group, an aryl group, an alkoxy group, an aryloxy group, a heterocyclic group, etc.

The sum of the number of the carbon atoms of R<sup>2</sup> and R<sup>3</sup> (including their substituents) is preferably 6 to 40.

In the above General Formulas (J-1) and (J-2), wherein R<sup>4</sup> to R<sup>13</sup> each represent a hydrogen atom, an alkyl group or an aryl group, the alkyl group represented by R<sup>4</sup> to R<sup>13</sup> may include, for example, a methyl group, an ethyl group, etc. The aryl group represented by R<sup>4</sup> to R<sup>13</sup> may include a phenyl group, etc.

General Formula (K)



In the formula, R<sup>1</sup> represents an aliphatic group, a cycloalkyl group or an aryl group, and Y represents a simple bond arm or a divalent hydrocarbon group necessary for forming a heterocyclic ring of 5 to 7 members together with a nitrogen atom. R<sup>2</sup>, R<sup>3</sup>, R<sup>4</sup>, R<sup>5</sup>, R<sup>6</sup> and R<sup>7</sup> each represent a hydrogen atom, an aliphatic group, a cycloalkyl group or an aryl group. However, R<sup>2</sup> and R<sup>4</sup>, and R<sup>3</sup> and R<sup>6</sup> each may be bonded to each other to form a simple bond arm to form an unsaturated heterocyclic ring of 5 to 7 members together with a nitrogen atom and Y. Also, when Y is a simple bond arm, R<sup>5</sup> and R<sup>7</sup> may be bonded to each other to form the simple bond arm to form an unsaturated heterocyclic ring of 5 to 7 members together with Y. When Y is not the simple bond arm, R<sup>5</sup> and Y, and R<sup>7</sup> and Y or Y itself may form unsaturated bonds to form an unsaturated heterocyclic ring of 6 or 7 members together with a nitrogen atom and Y.

The aliphatic group represented by R<sup>1</sup> may include a saturated alkyl group which may have a substituent and an unsaturated alkyl group which may have a substituent. The saturated alkyl group may include, for example, a methyl group, an ethyl group, a butyl group, an octyl group, a dodecyl group, a tetradecyl group, a hexadecyl group, etc., and the unsaturated alkyl group may include, for example, an ethenyl group, a propenyl group, etc.

The cycloalkyl group represented by R<sup>1</sup> may include a cycloalkyl group of 5 to 7 members which may have a substituent, for example, a cyclopentyl group, a cyclohexyl group, etc.

The aryl group represented by R<sup>1</sup> may include a phenyl group and a naphthyl group, each of which may have a substituent.

The substituents for the aliphatic group, the cycloalkyl group and the aryl group represented by R<sup>1</sup> may include an alkyl group, an aryl group, an alkoxy group, a carbonyl group, a carbamoyl group, an acylamino group, a sulfamoyl group, a sulfonamide group, a carbonyloxy group, an alkylsulfonyl group, an arylsulfonyl group, a hydroxyl group, a heterocyclic ring, an alkylthio group, an arylthio group, etc., and these substituents may further have a substituent.

In the above General Formula (K), wherein Y represents a simple bond arm or a divalent hydrocarbon group necessary for forming a heterocyclic ring of 5 to 7 members together with a nitrogen atom, and when Y is the simple bond arm, R<sup>5</sup> and R<sup>7</sup> may further be bonded to each other to form a simple bond arm to form an unsaturated heterocyclic ring of 5 members; when Y is the divalent hydrocarbon group, namely a methylene group, R<sup>5</sup> and Y, or R<sup>7</sup> and Y may form an unsaturated bond to form an unsaturated heterocyclic ring of 6

members, and when it is an ethylene group, R<sup>5</sup> and Y, R<sup>7</sup> and Y, or Y itself may form an unsaturated bond to form an unsaturated heterocyclic ring of 7 members. Further, the divalent hydrocarbon represented by Y may have a substituent, and such a substituent may include an alkyl group, a carbamoyl group, an alkyloxycarbonyl group, an acylamino group, a sulfonamide group, a sulfamoyl group, an aryl group, a heterocyclic group, etc.

In the above General Formula (K), wherein R<sup>2</sup>, R<sup>3</sup>, R<sup>4</sup>, R<sup>5</sup>, R<sup>6</sup> and R<sup>7</sup> each represent a hydrogen atom, an aliphatic group, a cycloalkyl group or an aryl group, the aliphatic group represented by R<sup>2</sup> to R<sup>7</sup> may include a saturated alkyl group which may have a substituent and an unsaturated alkyl group which may have a substituent. The saturated alkyl group may include, for example, a methyl group, an ethyl group, a butyl group, an octyl group, a dodecyl group, a tetradecyl group, a hexadecyl group, etc., and the unsaturated alkyl group may include, for example, an ethenyl group, a propenyl group, etc.

The cycloalkyl group represented by R<sup>2</sup> to R<sup>7</sup> may include a cycloalkyl group of 5 to 7 members which may have a substituent, for example, a cyclopentyl group, a cyclohexyl group, etc.

The aryl group represented by R<sup>2</sup> to R<sup>7</sup> may include a phenyl group and a naphthyl group, each of which may have a substituent.

The substituents for the aliphatic group, the cycloalkyl group and the aryl group represented by R<sup>2</sup> to R<sup>7</sup> may include an alkyl group, an aryl group, an alkoxy group, a carbonyl group, a carbamoyl group, an acylamino group, a sulfamoyl group, a sulfonamide group, a carbonyloxy group, an alkylsulfonyl group, an arylsulfonyl group, a hydroxyl group, a heterocyclic group, an alkylthio group, etc.

The compound represented by the above General Formula (K) is more preferable when it has a saturated heterocyclic ring of 5 to 7 members than when it has an unsaturated one.

As the anti-color-fading agent according to this invention, there can be used any compounds so far as they have the oxidation potential in the range mentioned above, but preferably used are water insoluble compounds in order for the effect of the invention to be sufficiently exhibited. The oxidation potential may be 0.95 (V)  $\leq$  Eox  $\leq$  1.50 (V), but preferably 1.00 (V)  $\leq$  Eox  $\leq$  1.45 (V), particularly preferably 1.00 (V)  $\leq$  Eox  $\leq$  1.40 (V).

25 Specific compounds of the anti-color-fading agent according to this invention are shown below, but this invention is by no means limited to these compounds.





(AO-6)

-continued



(AO-7)



(AO-8)



(AO-9)



(AO-10)



(AO-11)



(AO-12)



(AO-13)

-continued

(AO-14)



(AO-15)



(AO-16)



(AO-17)



(AO-18)



(AO-19)



(AO-20)



(AO-21)





-continued

(AO-22)



(AO-23)



(AO-24)



(AO-25)



(AO-26)



(AO-27)



(AO-28)



(AO-29)

The anti-color-fading agent according to this invention is added to the silver halide emulsion layer containing the magenta coupler represented by the above General Formula (I). The anti-color-fading agent according to this invention may be added in any amount depending on the intended effect and the kind of the compound, but it can be used preferably in an amount of 0.05 mole to 3 moles, more preferably 0.1 mole to 2

moles, per 1 mole of the magenta coupler of the invention, represented by the above General Formula (I).

The hydroquinone derivative used in this invention will be described below.

In this invention, preferably usable hydroquinone derivative may include the compounds represented by General Formulas (XII) and (XIII) or precursors thereof.



General Formula (XII)

In the formula, R<sup>1</sup> and R<sup>2</sup> each represent an alkyl group (for example, a butyl group, a pentyl group, an octyl group, etc.), an aryl group (for example, a phenyl group, etc.), an alkenyl group (for example, a propenyl group, a butenyl group, etc.), a cycloalkyl group (for example, a cyclohexyl group, etc.) or a heterocyclic group (for example, cumarone, etc.). Each of these groups may also include those having a substituent, which may include an alkyl group, an aryl group, etc.



General Formula (XIII)

In the formula, R<sup>3</sup> and R<sup>4</sup> each represent an alkyl group having 1 to 5 carbon atoms (for example, a methyl group, a propyl group, a pentyl group, etc.); R<sup>5</sup> represents an alkyl group (for example, a methyl group, a pentyl group, a dodecyl group, etc.), an aryl group (for example, a phenyl group, etc.), an alkenyl group (for example, a propenyl group, a butenyl group, etc.), a cycloalkyl group (for example, a cyclohexyl group, etc.), a heterocyclic group (for example, cumarone, etc.), or a group of:



wherein n represents an integer of 1 to 20; k is 1 or 2; and Q represents a group of —COXR<sup>6</sup> [wherein X represents an oxygen atom or a group of:



R<sup>6</sup> represents a hydrogen atom, an alkyl group (for example, a methyl group, a hexyl group, a dodecyl group, etc.), an alkenyl group (for example, a propenyl group, etc.), a cycloalkyl group (for example, a cyclohexyl group, etc.) or an aryl group (for example, a phenyl group, etc.); R<sup>7</sup> represents a hydrogen atom, an

alkyl group (for example, a methyl group, etc.) or an aryl group (for example, a phenyl group, etc.); and each of these group may include one having a substituent], a group of —OY (wherein Y represents —R<sup>6</sup> or —COR<sup>6</sup>), a group of:



10

(wherein R<sup>8</sup> represents a hydrogen atom, an alkyl group, an aryl group, or —COR<sup>6</sup>), a group of —P(O)(OR<sup>6</sup>)([O]IR<sup>9</sup>) (wherein R<sup>9</sup> has the same meaning as defined for R<sup>6</sup> and 1 is 0 or 1), or a cyano group.

Of the hydroquinone derivatives included in the compound represented by General Formula (XII), more preferable are those included in the compound represented by General Formula (XII') shown below or precursors thereof.



General Formula (XII')

25 In the formula, R<sup>10</sup> and R<sup>11</sup> each represent a hydrogen atom or an alkyl group having 1 to 5 carbon atoms, R<sup>6</sup> has the same meaning as defined for R<sup>6</sup> in General Formula (XIII), provided, however, that R<sup>10</sup> and R<sup>11</sup> are not a hydrogen atom at the same time.

30 Also, of the hydroquinone derivatives included in the compound represented by General Formula (XIII), more preferable are those included in the compound represented by General Formula (XIII') shown below or precursors thereof.



35 In the formula, R<sup>3</sup>, R<sup>4</sup>, R<sup>6</sup> and n have the same meaning as defined for R<sup>3</sup>, R<sup>4</sup>, R<sup>6</sup> and n in General Formula (XIII).

40 Specific examples of the hydroquinone derivatives 50 according to this invention are shown below, but this invention is by no means limited by these.



(HQ-1)

-continued



(HQ-2)



(HQ-3)



(HQ-4)



(HQ-5)



(HQ-6)



(HQ-7)



(HQ-8)



(HQ-9)



(HQ-10)

-continued



(HQ-11)



(HQ-12)



(HQ-13)



(HQ-14)



(HQ-15)



(HQ-16)



(HQ-17)



(HQ-18)

-continued



(HQ-19)



(HQ-20)



(HQ-21)



(HQ-22)



(HQ-23)



(HQ-24)



(HQ-25)

-continued



The hydroquinone derivative according to this invention may be used in any amount if added in the range of  $1 \times 10^{-3}$  mole to 0.1 mole per 1 mole of the magenta coupler of this invention, represented by the above General Formula (I), but preferably in amount ranging between  $5 \times 10^{-3}$  mole and 0.08 mole, particularly preferably  $5 \times 10^{-3}$  mole and 0.05 mole. The hydroquinone derivative according to this invention may be added to the silver halide emulsion layer containing the magenta coupler represented by the above General Formula (I), and may be further added to a layer or layers adjacent thereto, without any inconvenience.

Conventionally, the above hydroquinone derivatives are disclosed as anti-staining agents, in Research Disclosure Vol. 176 (1978), No. 17643, Paragraph VII-I, Japanese Unexamined Patent Publication Nos. 24141/1983, 25 180557/1984 and 189342/1984, etc.

As the method of adding the magenta coupler, anti-color-fading agent and hydroquinone derivative according to this invention to a light sensitive silver halide photographic material, there can be used a variety of methods such as a solid dispersion method, a latex dispersion method and an oil-in-water emulsification dispersion method, in the same manner as in the method generally carried out for adding hydrophobic compounds. This can be suitably selected depending on the chemical structure of the hydrophobic compounds such as couplers. As the oil-in-water emulsification dispersion method, a conventionally known method for dispersing hydrophobic additives such as couplers can be applied. Usually, the method may be carried out by dissolving the couplers in a high boiling organic solvent having a boiling point of 150° C. or more optionally together with a low boiling and/or water soluble organic solvent, and carrying out emulsification dispersion in a hydrophilic binder such as an aqueous gelatin solution by use of a surface active agent and by use of a dispersing means such as a stirrer, a homogenizer, a colloid mill, a flow jet mixer, an ultrasonic device, followed by adding the dispersion to an intended hydrophilic colloid layer. There may be inserted a step of removing the dispersing solution or, at the same time of the dispersion, the low boiling organic solvent.

The high boiling solvent to be used may include organic solvents having a boiling point of 150° C. or more such as phenol derivatives, phthalates, phosphates, citrates, benzoates, alkyl amides, aliphatic acid esters and trimesic acid esters which do not react with an oxidized product of a developing agent.

In this invention, the high boiling organic solvent which can be preferably used in dispersing the compounds such as the anti-color-fading agent and hydroquinone derivative according to this invention is a compound having a dielectric constant of 6.0 or less, including, for example, esters such as phthalates and phosphates, organic amides, ketones, hydrocarbon compounds, etc. having the dielectric constant of 6.0 or less. Preferred are high boiling organic solvents having a dielectric constant of not more than 6.0 and not less

(HQ-26)

than 1.9, and having a vapor pressure of 0.5 mmHg or less at 100° C. More preferred are phthalates or phosphates among the above high boiling organic solvents. The high boiling organic solvent may also be a mixture of two or more kinds.

The dielectric constant mentioned in this invention refers to the dielectric constant at 30° C.

The phthalates that can be advantageously used in this invention may include the compound represented by General Formula (a) shown below:



General Formula (a)

In the formula, R<sup>1</sup> and R<sup>2</sup> each represent an alkyl group, an alkenyl group or an aryl group, provided, however, that the sum of carbon atom numbers of the groups represented by R<sup>1</sup> and R<sup>2</sup> is 8 to 32. More preferably, the sum of the carbon atom numbers is 16 to 24.

In this invention, the alkyl group represented by R<sup>1</sup> and R<sup>2</sup> in the above General Formula (a) may be straight chain or branched one, including, for example, a butyl group, a pentyl group, a hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, an octadecyl group, etc. The aryl group represented by R<sup>1</sup> and R<sup>2</sup> may include, for example, a phenyl group, a naphthyl group, etc.; the alkenyl group may include, for example, a hexenyl group, a heptenyl group, an octadecenyl group. These alkyl group, alkenyl group and aryl group may have a single or plural number of substituent(s), and the substituent for the alkyl group and the alkenyl group may include, for example, a halogen atom, an alkoxy group, an aryl group, an aryloxy group, an alkenyl group, an alkoxy carbonyl group, etc., and the substituent for the aryl group may include, for example, a halogen atom, an alkyl group, an alkoxy group, an aryl group, an aryloxy group, an alkenyl group, an alkoxy carbonyl group, etc.

The phosphates that can be advantageously used in this invention may include those represented by General Formula (b) shown below:



General Formula (b)

In the formula, R<sup>3</sup>, R<sup>4</sup> and R<sup>5</sup> each represent an alkyl group, an alkenyl group or an aryl group, provided, however, that the sum of the carbon atom numbers of the groups represented by R<sup>3</sup>, R<sup>4</sup> and R<sup>5</sup> is 24 to 54.

101

The alkyl group represented by  $R^3$ ,  $R^4$  and  $R^5$  in General Formula (b) may include, for example, a butyl group, a pentyl group, a hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, an octadecyl group, a nonadecyl group, etc.; the aryl group may include, for example, a phenyl group, a naphthyl group, etc.; and the alkenyl group may include, for example, a hexenyl group, a heptenyl group, an octadecenyl group, etc.

These alkyl group, alkenyl group and aryl group may have a single or plural number of substituent(s). Preferably,  $R^3$ ,  $R^4$  and  $R^5$  each represent an alkyl group, including, for example, a 2-ethylhexyl group, a n-octyl group, a 3,5,5-trimethylhexyl group, a n-nonyl group, a n-decyl group, a sec-decyl group, a sec-dodecyl group, a t-octyl group, etc.

Typical examples of the organic solvents used in this invention are shown below, but this invention is by no means limited to these.

Exemplary organic solvents:



5

15

20

25

30

35

40

45

50

55

60

65

102



S-8



S-9



S-10



S-11



S-12



S-13



S-14



S-15



S-16



S-17



S-18



S-19



S-20

-continued



These organic solvents may be used generally in the proportion of 10 to 150% by weight based on the magenta coupler of this invention, and, preferably, 20 to 100% by weight based on the coupler.

As a dispersion auxiliary, used when dissolving the hydrophobic compounds such as couplers in a solvent comprising the organic solvent alone or the combination thereof with a low boiling solvent to effect dispersion in water by use of a mechanical or ultrasonic means, there can be used anionic surface active agents, nonionic surface active agents, and cationic surface active agents.

The light-sensitive silver halide photographic material of this invention includes, for example, color negative and positive films and color photographic papers, and the effect of this invention can be effectively exhibited when the color photographic papers for direct appreciation are used.

The light-sensitive silver halide photographic material including the color photographic papers may be those for either monicolor or multicolor. In the case of the multicolor light-sensitive silver halide photographic material, wherein the color reproduction is carried out by the subtractive color process, the photographic material usually has the construction comprising silver halide emulsion layers respectively containing magenta, yellow and cyan couplers as couplers for photography, and non-sensitive layers, laminated on a support with an appropriate number and order of layers. The number and order of the layers may be suitably changed depending on what performances are important and what purpose the materials are used for.

In the case where the light-sensitive silver halide photographic material is the multicolor light-sensitive silver halide photographic material, specific layer constitution is particularly preferably such that, from the support side, a yellow dye image forming layer, an intermediate layer, a magenta dye image forming layer, an intermediate layer, a cyan dye image forming layer, an intermediate layer and a protective layer are successively arranged on the support.

In the silver halide emulsion used in the light-sensitive silver halide photographic material of this invention, there can be used any of silver bromide, silver iodobromide, silver iodochloride, silver chlorobromide, silver chloride, etc. which are used in ordinary silver halide emulsions.

Silver halide grains used in the silver halide emulsions may be obtained by any of an acidic method, a neutral method and an ammoniacal method. The grains may be allowed to grow at one time, or grow after seed grains have been formed. The manner to prepare the seed grains and the manner to grow them may be same or different.

The silver halide emulsion may be obtained by simultaneously mixing halide ions and silver ions, or by preparing an aqueous solution in which either one of them is present and then mixing in it the other of them. Alternatively, taking into account the critical growth rate of silver halide crystals, it may be formed by successively simultaneously adding halide ions and silver ions while controlling pH and pAg in a mixing vessel. Halogen formulation in a grain may be varied after growth by employing a conversion method.

During the preparation of the silver halide emulsion of this invention, a silver halide solvent can be optionally used for controlling the grain size, grain shape, grain size distribution and grain growth rate, of the silver halide grains.

In the course of formation and/or growth of the silver halide grains used in the silver halide emulsion of this invention, metal ions may be added to the grains by use of at least one of a cadmium salt, a zinc salt, a lead salt, a thallium salt, an iridium salt or a complex salt thereof, a rhodium salt or a complex salt thereof, and an iron salt or a complex salt thereof to incorporate any of these metal elements into the inside of the grains and/or the surface of the grains, and also a reduction sensitizing nuclei can be imparted to the inside of the grains and/or the surface of the grains by placing the grains in a suitable reductive atmosphere.

The silver halide emulsion may be either one from which unnecessary soluble salts have been removed after completion of the growth of silver halide grains, or one from which they remain unremoved. When the salts are removed, they can be removed according to the method disclosed in Research Disclosure No. 17643.

The silver halide grains used in the silver halide emulsion of this invention may comprise uniform layers in the inside and the surface, or comprise different layers.

The silver halide grains used in the silver halide emulsion of this invention may be grains such that a latent image is formed chiefly on the surface, or grains such that a latent image is formed chiefly in the inside of a grain.

The silver halide grains used in the silver halide emulsion of this invention may be any of those having a regular crystal form, or those having an irregular crystal form such as a sphere and a plate. In these grains, there can be used those having any ratio of {100} face to {111} face. Also, they may have a composite form of these crystal forms, or comprise a mix of grains having various crystal forms.

The silver halide emulsion may be used by mixing two or more kinds of silver halide emulsions which have been separately formed.

The silver halide emulsion can be chemically sensitized according to conventional methods. Namely, a sulfur sensitization method using a compound containing sulfur capable of reacting with silver ions, and active gelatin, a selenium sensitization method using a selenium compound, a reduction sensitization method using a reducing substance, and a noble metal sensitization method using noble metal compounds such as gold and so forth can be used alone or in combination.

The silver halide emulsion of this invention can be optically sensitized to a desired wavelength region by using a dye known as a sensitizing dye in the field of photography. The sensitizing dye may be used alone, or may be used in combination of two or more of the dye. Together with the sensitizing dye, a dye having itself no action of spectral sensitization, or a supersensitizing

agent which is a compound substantially absorbing no visible light and capable of strengthening the sensitizing action of the sensitizing dye, may be contained in the emulsion.

To the silver halide emulsion of this invention, a compound known as an antifogger or a stabilizer in the field of photography can be added during chemical ripening, and/or after completion of chemical ripening, and/or before coating of a silver halide emulsion after completion of chemical ripening, for the purpose of preventing a light-sensitive material from being fogged during production of light-sensitive materials, during preservation or during photographic processing, or for the purpose of keeping stable the photographic performances.

As a binder (or a protective colloid) for the silver halide emulsion of this invention, it is advantageous to use gelatin, but it is also possible to use hydrophilic colloids such as gelatin derivatives, a graft polymer of gelatin with other macromolecules, proteins, sugar derivatives, cellulose derivatives and synthetic hydrophilic high molecular substances such as homopolymer or copolymer.

Photographic emulsion layers and other hydrophilic colloid layers of the light-sensitive material in which the silver halide emulsion of this invention is used can be hardened by using one or more kinds of hardening agents that can crosslink binder (or protective colloid) molecules to enhance the film strength. The hardening agents can be added in such an amount that a light-sensitive material can be hardened to the extent that no hardening agent is required to be added in a processing solution. It, however, is also possible to add the hardening agent in the processing solution.

A plasticizer can be added to the silver halide emulsion layers and/or other hydrophilic colloid layers of the light-sensitive material, in which the silver halide emulsions of this invention are used, for the purpose of enhancing flexibility.

For the purpose of improving dimensional stability and the like, a dispersion (latex) of a water insoluble or hardly soluble synthetic polymer can be contained in the photographic emulsion layers and other hydrophilic colloid layers in which the silver halide emulsions of this invention are used.

In a color development processing, a dye-forming coupler capable of forming a dye through a coupling reaction with an oxidized product of an aromatic primary amine developing agent (for example, p-phenylenediamine derivatives, aminophenol derivatives, etc.) is used in the emulsion layers of the light-sensitive material of this invention. In a usual case, the dye forming coupler is selected in the manner that there can be formed a dye capable of absorbing light-sensitive spectral light in an emulsion layer with respect to the respective emulsion layers, and thus a yellow dye-forming coupler is used in a blue-sensitive emulsion layer; a magenta dye-forming coupler, in a green-sensitive emulsion layer; and a cyan dye-forming coupler, in a red-sensitive emulsion layer. However, the light-sensitive silver halide color photographic material may be prepared by using the couplers in the manner different from the above combination, depending on the purpose.

The cyan dye-forming coupler used in this invention may typically include four equivalent type or two equivalent type phenol or naphthol cyan dye-forming couplers, and Specific examples are disclosed in U.S. Pat. Nos. 2,306,410, 2,356,475, 2,362,598, 2,367,531,

5 2,369,929, 2,423,730, 2,474,293, 2,476,008, 2,498,466, 2,545,687, 2,728,660, 2,772,162, 2,895,826, 2,976,146, 3,002,836, 3,419,390, 3,446,622, 3,476,563, 3,737,316, 3,758,308, and 3,839,044; British Patent Nos. 478,991, 945,542, 1,084,480, 1,377,237, 1,388,024 and 1,543,040; Japanese Unexamined Patent Publication Nos. 37425/1972, 10135/1975, 25228/1975, 112038/1975, 117422/1975, 130441/1975, 6551/1976, 37647/1976, 52828/1976, 108841/1976, 109630/1978, 48237/1979, 66129/1979, 131931/1979 and 32071/1980; etc.

10 Cyan couplers used in this invention may preferably further include those represented by General Formula (C-1) and (C-2) shown below:

15

General Formula (C-1)



20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

General Formula (C-1)



General Formula (C-2)

In the formula, R<sup>1</sup> represents an alkyl group or an aryl group. R<sup>2</sup> represents an alkyl group, a cycloalkyl group, an aryl group or a heterocyclic group. R<sup>3</sup> represents a hydrogen atom, a halogen atom, an alkyl group or an alkoxy group. R<sup>4</sup> may be linked with R<sup>1</sup> to form a ring. Z represents a hydrogen atom or a group eliminable through the reaction with an oxidized product of an aromatic primary amine type color developing agent.

In the formula, R<sup>4</sup> represents a straight chain or branched alkyl group having 1 to 4 carbon atoms, and R<sup>5</sup> represents a ballast group. Z has the same meaning as defined for Z in General Formula (C-1). Particularly preferably R<sup>4</sup> represents a straight chain or branched alkyl group having 2 to 4 carbon atoms.

In this invention, the alkyl group represented by R<sup>1</sup> in General Formula (C-1) is straight chain or branched one, including, for example, a methyl group, an ethyl group, an iso-propyl group, a butyl group, a pentyl group, an octyl group, a nonyl group, a tridecyl group, etc., and the aryl group include, for example, a phenyl group, a naphthyl group, etc. These groups represented by R<sup>1</sup> may include those having a single or plural number of substituent(s), and the substituent(s) introduced, for example, in the phenyl group may typically include halogen atoms (for example, atoms of fluorine, chlorine, bromine, etc.), alkyl groups (for example, a methyl group, an ethyl group, a propyl group, a butyl group, a dodecyl group, etc.), hydroxyl groups, cyano groups, nitro groups, alkoxy groups (for example, a methoxy group and an ethoxy group), alkylsulfonamide groups (for example, a methylsulfonamide group, an octylsulfonamide group, etc.), arylsulfonamide groups (for example, a phenylsulfonamide group, a naphthylsulfonamide group, etc.), alkylsulfamoyl groups (for example, butylsulfamoyl group, etc.), arylsulfamoyl groups (for example, a phenylsulfamoyl group, etc.), alkyloxycarbonyl groups (for example, a methyloxycarbonyl group,

etc.), aryloxycarbonyl groups (for example, a phenyloxycarbonyl group, etc.), aminosulfonamide groups (for example, N,N-dimethylaminosulfonamide group, etc.), acylamino groups, carbamoyl groups, sulfonyl groups, sulfinyl groups, sulfoxy group, sulfo groups, aryloxy groups, alkoxy groups, carboxyl groups, alkylcarbonyl groups, arylcarbonyl groups, etc.

Two or more of these substituents may be introduced in the phenyl group.

The halogen atom represented by R<sup>3</sup> may include, for example, a fluorine atom, a chlorine atom, a bromine atom, etc.; the alkyl group may include, for example, a methyl group, an ethyl group, a propyl group, a butyl group, a dodecyl group, etc.; and the alkoxy group may include, for example, a methoxy group, an ethoxy group, a propyloxy group, a butoxy group, etc. R<sup>3</sup> may be linked with R<sup>1</sup> to form a ring.

In this invention, the alkyl group represented by R<sup>2</sup> in General Formula (C-1) includes, for example, a methyl group, an ethyl group, a butyl group, a hexyl group, a tridecyl group, a pentadecyl group, a heptadecyl group, a so called polyfluoroalkyl group which is a group substituted with a fluorine atom, etc.

The aryl group represented by R<sup>2</sup> includes, for example, a phenyl group and naphthyl group and preferably includes a phenyl group. The heterocyclic group represented by R<sup>2</sup> includes, for example, a pyridyl group, a furan group, etc. The cycloalkyl group represented by R<sup>2</sup> includes, for example, a cyclopropyl group, a cyclohexyl group, etc. These groups represented by R<sup>2</sup> may include those having a single or plural number of substituent(s), and the substituent(s) introduced, for example, in the phenyl group may typically include halogen atoms (for example, atoms of fluorine, chlorine, bromine, etc.), alkyl groups (for example, a methyl group, an ethyl group, a propyl group, a butyl group, a dodecyl group, etc.), hydroxyl groups, cyano groups, nitro groups, alkoxy groups (for example, a methoxy group and an ethoxy group), alkylsulfonamide groups (for example, a methylsulfonamide group, an octylsulfonamide group, etc.), arylsulfonamide groups (for example, a phenylsulfonamide group, a naphthylsulfonamide group, etc.), alkylsulfamoyl groups (for example, butylsulfamoyl group, etc.), arylsulfamoyl groups (for example, a phenylsulfamoly group, etc.), alkyloxycarbonyl groups (for example, a methyloxycarbonyl group, etc.), aryloxycarbonyl groups (for example, a phenyloxycarbonyl group, etc.), aminosulfonamide groups (for example, N,N-dimethylaminosulfonamide group, etc.), acylamino groups, carbamoyl groups, sulfonyl groups, sulfinyl groups, sulfoxy group, sulfo groups, aryloxy groups, alkoxy groups, carboxyl groups, alkylcarbonyl groups, arylcarbonyl groups, etc. Two or more of these substituents may be introduced in the phenyl group.

The group represented by R<sup>9</sup> may preferably include a polyfluoroalkyl group, a phenyl group, or a phenyl group having as a substituent one or more of a halogen atom, an alkyl group, an alkoxy group, an alkylsulfonamide group, an arylsulfonamide group, an alkylsulfamoyl group, an arylsulfamoyl group, an alkylsulfonyl group, an arylsulfonyl group, an alkylcarbonyl group, an arylcarbonyl group and a cyano group.

The cyan couplers represented by the above General Formula (C-1) and preferably used in this invention, may further preferably include those represented by General Formula (C-3) shown below.

General Formula (C-3)



10

In General Formula (C-3), R<sup>6</sup> represents a phenyl group. This phenyl group may include one having a single or plural number of substituent(s), and the substituent(s) introduced therein may typically include halogen atoms (for example, atoms of fluorine, chlorine, bromine, etc.), alkyl groups (for example, a methyl group, an ethyl group, a propyl group, a butyl group, a dodecyl group, etc.), hydroxyl groups, cyano groups, nitro groups, alkoxy groups (for example, a methoxy group and an ethoxy group), alkylsulfonamide groups (for example, a methylsulfonamide group, an octylsulfonamide group, etc.), arylsulfonamide groups (for example, a phenylsulfonamide group, a naphthylsulfonamide group, etc.), alkylsulfamoyl groups (for example, butylsulfamoyl group, etc.), arylsulfamoyl groups (for example, a phenylsulfamoly group, etc.), alkyloxycarbonyl groups (for example, a methyloxycarbonyl group, etc.), aryloxycarbonyl groups (for example, a phenyloxycarbonyl group, etc.), etc. Two or more of these substituents may be introduced in the phenyl group.

The group represented by R<sup>6</sup> may preferably include a phenyl group, or a phenyl group having as a substituent one or more of a halogen atom (preferably fluorine, chlorine or bromine), an alkylsulfonamide group (preferably an o-methylsulfonamide group, a p-octylsulfonamide group or an o-dodecylsulfonamide group), an arylsulfonamide group (preferably a phenylsulfonamide group), an alkylsulfamoyl group (preferably a butylsulfamoyl group), an arylsulfamoyl group (preferably a phenylsulfamoyl group), an alkyl group (preferably a methyl group or trifluoromethyl group) and an alkoxy group (preferably a methoxy group or an ethoxy group).

R<sup>7</sup> is an alkyl group or an aryl group. The alkyl group or the aryl group may include those having a single or plural number of substituent(s), and the substituent(s) thereof may typically include halogen atoms (for example, fluorine, chlorine, bromine, etc.), hydroxyl groups, carboxyl groups, alkyl groups (for example, a methyl group, an ethyl group, a propyl group, a butyl group, a dodecyl group, a benzyl group, etc.), cyano groups, nitro groups, alkoxy groups (for example, a methoxy group and an ethoxy group), aryloxy group, alkylsulfonamide groups (for example, a methylsulfonamide group, an octylsulfonamide group, etc.), arylsulfonamide groups (for example, a phenylsulfonamide group, a naphthylsulfonamide group, etc.), alkylsulfamoyl groups (for example, butylsulfamoyl group, etc.), arylsulfamoyl groups (for example, a phenylsulfamoly group, etc.), alkyloxycarbonyl groups (for example, a methyloxycarbonyl group, etc.), aryloxycarbonyl groups (for example, a phenyloxycarbonyl group, etc.), aminosulfonamide groups (for example, dimesitylaminosulfonamide group, etc.), alkylsulfonyl groups, arylsulfonyl groups, alkylcarbonyl groups, arylcarbonyl groups, aminocarbonylamide groups, carbam-

oyl groups, sulfinyl groups, etc. Two or more of these substituents may be introduced.

The group represented by  $R^7$  may preferably include an alkyl group when  $n^1=0$ , or an aryl group when  $n^1=1$  or more. The group represented by  $R^7$  may further preferably include an alkyl group having 1 to 22 carbon atoms when  $n^1=0$  (preferably a methyl group, an ethyl group, a propyl group, a butyl group, an octyl group or a dodecyl group), or, when  $n^1=1$  or more, an unsubstituted phenyl group or a phenyl group having as a substituent one or more of an alkyl group (preferably a t-butyl group, a t-amyl group or an octyl group), an alkylsulfonamide group (preferably a butylsulfonamide group, an octylsulfonamide group or a dodecylsulfonamide group), an arylsulfonamide group (preferably a phenylsulfonamide group), an aminosulfonamide group (preferably a dimethylaminosulfonamide group) and an alkyloxycarbonyl group (preferably a methyloxycarbonyl group or a butyloxycarbonyl group).

$R^8$  represents an alkylene group, preferably a straight chain or branched alkylene group having 1 to 20 carbon atoms, more preferably 1 to 12 carbon atoms.

$R^9$  represents a hydrogen atom or a halogen atom (fluorine, chlorine, bromine or iodine). Preferably, it is a hydrogen atom.

$n^1$  is 0 or a positive integer, preferably 0 or 1.

$X$  represents a divalent group of a group of  $—O—$ ,  $—CO—$ ,  $—COO—$ ,  $—OCO—$ ,  $—SO_2NR'—$ ,  $—NR'—SO_2NR''—$ ,  $—S—$ ,  $—SO—$  or  $—SO_2—$  (herein,  $R'$ ,  $R''$  and  $R'''$  each represent an alkyl group and include those having a substituent). Preferably,  $X$  is a group of  $—O—$ ,  $—S—$ ,  $—SO—$  or  $—SO_2—$ .

$Z$  has the same meaning as defined for  $Z$  in General Formula (C-1).

In this invention, the straight chain or branched alkyl group having 1 to 4 carbon atoms, represented by the above General Formula (C-2) is, for example, an ethyl group, a propyl group, a butyl group, an iso-propyl group, an iso-butyl group, a sec-butyl group or a tert-butyl group, and may include those having a substituent. The substituent may include an acylamino group (for example, an acetylamino group), an alkoxy group (for example a methoxy group), etc.

Preferably,  $R^4$  is an alkyl group having 2 to 4 carbon atoms.

The ballast group represented by  $R^5$  is an organic group having the size and shape that can give to a coupler molecule the bulk sufficient for making it substantially impossible for the coupler to be diffused to other layer from a layer to which the coupler is applied.

Typical ballast group may include an alkyl group having 8 to 32 carbon atoms in total, or an aryl group.

These alkyl group or aryl group may include those having a substituent. The substituent for the aryl group may include, for example, an alkyl group, an aryl group, an alkoxy group, an aryloxy group, a carboxyl group, an acyl group, an ester group, a hydroxyl group, a cyano group, a nitro group, a carbamoyl group, a carbonamide group, an alkylthio group, an arylthio group, a sulfonyl group, a sulfonamide group, a sulfamoyl group and a halogen atom. Also, the substituent for the alkyl group may include the substituents set forth for the above aryl group, except an alkyl group.

Particularly preferable ballast group may include the compound represented by General Formula (C-4) shown below.



General Formula (C-4)

$R^{10}$  represents a hydrogen atom or an alkyl group having 1 to 12 carbon atoms,  $Ar$  represents an aryl group such as a phenyl group, and the aryl group may include one having a substituent. The substituent may include an alkyl group, a hydroxyl group, an alkylsulfonamide group, etc., and most preferable one includes a branched alkyl group such as t-butyl group.

In General Formulas (C-1) and (C-2), the groups eliminable through the reaction with an oxidized product of an aromatic primary amine type color developing agent, each represented by  $Z$ , may include those known to a person skilled in the art, and also those which may advantageously act as modifying the reactivity of a coupler, or being eliminated from a coupler to achieve functions such as development restraint, bleach restraint and color correction in the coated layers containing the coupler or other layers in a light-sensitive silver halide color photographic material. Typically, they may include, for example, a halogen atom typified by chlorine and fluorine, an alkoxy group, an aryloxy group, an arylthio group, a carbamoyloxy group, an acyloxy group, a sulfonyloxy group, a sulfonamide group, or a heteroarylthio group, a heteroaryloxy group, etc.  $Z$  is particularly preferably a hydrogen atom or a chlorine atom.

More specifically, they are disclosed in Japanese Unexamined Patent Publications Nos. 10135/1975, 120334/1975, 130441/1975, 48237/1979, 146828/1976, 14736/1979, 37425/1972, 123341/1975 and 95346/1983; Japanese Patent Publications No. 36894/1973; U.S. Pat. Nos. 3,476,563, 3,737,316 and 3,227,551.

Typical examples of the cyan couplers represented by General Formula (C-1) are shown below, but by no means limited to these.



-continued



C-2



C-3



C-4



C-5



C-6



C-7



C-8



C-9



C-10



C-11



C-12



C-13



C-14



C-15

(n)C<sub>12</sub>H<sub>25</sub>SO<sub>2</sub>NH

-continued



C-16



C-17



C-18



C-19



C-20



C-21



C-22



-continued



C-23



C-24



C-25



C-26



C-27



C-28



C-29

-continued



Typical examples of the cyan couplers represented by General Formula (C-2) are shown below, but by no means limited to these.

---

General Formula (C-2)



| Coupler No. | $R^4$            | $Z$                              | $R^5$                                                           |
|-------------|------------------|----------------------------------|-----------------------------------------------------------------|
| C-33        | $-C_2H_5$        | $-Cl$                            | $tC_5H_{11}$<br>$-CH_2O-$<br>$tC_5H_{11}-tC_5H_{11}$            |
| C-34        | $-C_2H_5$        | $-O-$<br>$C_6H_4-$<br>$NHCOCH_3$ | $tC_5H_{11}$<br>$-CHO-$<br>$C_2H_5-$<br>$tC_5H_{11}-tC_5H_{11}$ |
| C-35        | $CH_3$<br>$CH_3$ | $-Cl$                            | $-CHO-$<br>$C_2H_5-$<br>$C_{15}H_{31}$                          |

-continued

## General Formula (C-2)



| Coupler No. | R <sup>4</sup>                     | Z   | R <sup>5</sup>                   |
|-------------|------------------------------------|-----|----------------------------------|
| C-36        | —C <sub>2</sub> H <sub>5</sub>     | —Cl |                                  |
| C-37        | —C <sub>2</sub> H <sub>5</sub>     | —Cl |                                  |
| C-38        | —C <sub>4</sub> H <sub>9</sub>     | —F  |                                  |
| C-39        | —C <sub>2</sub> H <sub>5</sub>     | —F  |                                  |
| C-40        | —C <sub>2</sub> H <sub>5</sub>     | —Cl |                                  |
| C-41        | —C <sub>2</sub> H <sub>5</sub>     | —F  |                                  |
| C-42        | —CH <sub>3</sub>                   | —Cl |                                  |
| C-43        | —C <sub>2</sub> H <sub>5</sub>     | —Cl |                                  |
| C-44        | —C <sub>2</sub> H <sub>5</sub>     | —Cl |                                  |
| C-45        | —CH(CH <sub>3</sub> ) <sub>2</sub> | —Cl | —C <sub>18</sub> H <sub>37</sub> |

-continued

## General Formula (C-2)



| Coupler No. | R <sup>4</sup>                                        | Z   | R <sup>5</sup> |
|-------------|-------------------------------------------------------|-----|----------------|
| C-46        | —C <sub>2</sub> H <sub>5</sub>                        | —F  |                |
| C-47        | —CH <sub>3</sub>                                      | —Cl |                |
| C-48        | —C <sub>2</sub> H <sub>5</sub>                        | —Cl |                |
| C-49        | —C <sub>3</sub> H <sub>7</sub>                        | —Cl |                |
| C-50        | —C <sub>3</sub> H <sub>7</sub>                        | —Cl |                |
| C-51        | —C <sub>2</sub> H <sub>4</sub> NHC(=O)CH <sub>3</sub> | —Cl |                |
| C-52        | —C <sub>3</sub> H <sub>6</sub> OCH <sub>3</sub>       | —Cl |                |
| C-53        | —C <sub>2</sub> H <sub>5</sub>                        | —Cl |                |
| C-54        | —C <sub>2</sub> H <sub>5</sub>                        | —Cl |                |

-continued

## General Formula (C-2)



## Coupler

No.

R<sup>4</sup>

Z

R<sup>5</sup>

|      |  |  |  |
|------|--|--|--|
| C-55 |  |  |  |
| C-56 |  |  |  |
| C-57 |  |  |  |
| C-58 |  |  |  |
| C-59 |  |  |  |
| C-60 |  |  |  |
| C-61 |  |  |  |
| C-62 |  |  |  |
| C-63 |  |  |  |

-continued

### General Formula (C-2)



| Coupler<br>No. | R <sup>4</sup>                 | Z   | R <sup>5</sup>                                                                     |
|----------------|--------------------------------|-----|------------------------------------------------------------------------------------|
| C-64           | —C <sub>2</sub> H <sub>5</sub> | —Cl |  |

The yellow dye-forming couplers used in this invention may preferably include the compounds represented by General Formula (Y) shown below.



### General Formula (Y)

In the formula,  $R^{11}$  represents an alkyl group (for example, a methyl group, an ethyl group, a propyl group, a butyl group, etc.) or an aryl group (for example, a phenyl group, a p-methoxyphenyl group, etc.);  $R^{12}$  represents an aryl group; and  $Y^1$  represents a hydrogen atom or a group eliminable through the course of the color development reaction.

Further, particularly preferably dye-forming yellow couplers according to this invention may include the compounds represented by General Formula (Y') shown below.



In the formula,  $R^{13}$  represents a halogen atom, an alkoxy group or an aryloxy group;  $R^{14}$ ,  $R^{15}$ ,  $R^{16}$  and  $R^{17}$  each represents a hydrogen atom, a halogen atom, an alkyl group, an alkenyl group, an alkoxy group, an aryl group, an aryloxy group, a carbonyl group, a sulfonyl group, a carboxyl group, an alkoxy carbonyl group, a carbamyl group, a sulfone group, a sulfamyl group, a sulfonamide group, an acylamide group, an ureido group or an amino group; and  $Y^1$  has the same meaning as defined before.

$R^{13}$  is preferably a halogen atom, and  $R^{17}$  is preferably a hydrogen atom.

These compounds are disclosed in U.S. Pat. Nos. 2,778,658, 2,875,057, 2,908,573, 3,227,155, 3,227,550, 3,253,924, 3,265,506, 3,277,155, 3,341,331, 3,369,895, 3,384,657, 3,408,194, 3,415,652, 3,447,928, 3,551,155, 3,582,322, 3,725,072 and 3,894,875; German Unexamined Patent Publication Nos. 1,547,868, 2,057,941, 2,162,899, 2,163,812, 2,213,461, 2,219,917, 2,261,361 and 2,263,875; Japanese Patent Publication No. 13576/1974; Japanese Unexamined Patent Publications Nos. 29432/1973, 66834/1973, 10736/1974, 122335/1974, 28834/1975 and 132926/1975; etc.

Specific examples of the yellow couplers preferably used in this invention are shown below, but this invention is by no means limited to these.



-continued

Y-2



Y-3



Y-4



Y-5



Y-6



Y-7



-continued

Y-8



Y-9



Y-10



Hydrophilic colloid layer such as protective layers and intermediate layers of the light-sensitive material of this invention may contain an ultraviolet absorbent in order to prevent the fog due to the discharge caused by static charge by friction or the like of light-sensitive materials and prevent the deterioration due to ultraviolet light.

The light-sensitive silver halide material using the silver halide emulsion of this invention can be provided with auxiliary layer such as a filter layer, an anti-halation layer and an ant-irradiation layer. These layers and/or the emulsion layers may contain a dye that may be flowed out of the light-sensitive material, or bleached, during the development processing.

To the silver halide emulsion layers and/or other hydrophilic colloid layers of the light-sensitive material using the silver halide emulsion of this invention, a matte agent can be added for the purposes of decreasing the gloss of the light-sensitive material, improving the writing performance, and preventing mutual sticking of light-sensitive materials.

A lubricant can be added to the light-sensitive material using the silver halide emulsion of this invention, in order to decrease sliding friction.

An antistatic agent aiming at preventing static charge can be added to the light-sensitive material using the silver halide emulsion of this invention. The antistatic

agent may be used in an antistatic layer provided on the side of a support at which no emulsion layer is laminated, or may be used in an emulsion layer and/or a protective colloid layer other than the emulsion layers provided on the side of a support on which emulsion layers are laminated.

In the photographic emulsion layers and/or other hydrophilic colloid layers of the light-sensitive material using the silver halide emulsion of this invention, a variety of surface active agents can be used for the purpose of improving coating performance, preventing static charge, improving slidability, emulsification dispersion, preventing adhesion, and improving photographic performances (such as development acceleration, hardening and sensitization).

The support used in the light-sensitive material using the silver halide emulsion of this invention can be applied on flexible reflective supports made of baryta paper, paper laminated with  $\alpha$ -olefin polymers or synthetic paper; films comprising semisynthetic or synthetic high molecular compounds such as cellulose acetate, cellulose nitrate, polystyrene, polyvinyl chloride, polyethylene terephthalate, polycarbonate and polyamide; rigid bodies such as glass, metals and ceramics; etc.

The light-sensitive material of this invention may be applied, as occasion calls, after having been subjected to

corona discharging, ultraviolet irradiation, flame treatment and so forth, directly on the surface of the support or through interposition of one or more subbing layers for improving adhesion, antistatic performance, dimensional stability, abrasion resistance, hardness, anti-halation performance, friction characteristics and/or other characteristics of the surface of the support.

In the coating of the light-sensitive material, using the silver halide emulsion of this invention, a thickening agent may be used in order to improve the coating performance. Particularly useful coating method may include extrusion coating and curtain coating by which two or more layers can be simultaneously coated.

The light-sensitive material of this invention can be exposed by use of electromagnetic wave having the spectral region to which the emulsion layers constituting the light-sensitive material of this invention have the sensitivity. As a light source, there can be used any known light sources including natural light (sunlight), a tungsten lamp, a fluorescent lamp, a mercury lamp, a xenon arc lamp, a carbon arc lamp, a xenon flash lamp, a cathode ray tube flying spot, every kind of laser beams, light from a light-emitting diode, light emitted from a fluorescent substance energized by electron rays, X-rays, gamma-rays, alpha-rays, etc.

As for the exposure time, it is possible to make exposure, not to speak of exposure of 1 millisecond to 1 second usually used in cameras, of not more than 1 microsecond, for example, 100 microseconds to 1 microsecond by use of a cathode ray tube or a xenon arc lamp, and it is also possible to make exposure longer than 1 second. Such exposure may be carried out continuously or may be carried out intermittently.

The light-sensitive silver halide material of this invention can form images by carrying out color development known in the art.

The aromatic primary amine type color developing agent used for a color developing solution in this invention includes known ones widely used in the various color photographic processes. These developing agents include aminophenol type and p-phenylenediamine type derivatives. These compounds, which are more stable than in a free state, are used generally in the form of a salt, for example, in the form of a hydrochloride or a sulfate. Also, these compounds are used generally in concentration of about 0.1 to 30 g per 1 liter of a color developing solution, preferably in concentration of about 1 to 15 g per 1 liter of a color developing solution.

The aminophenol type developing agent may include, for example, o-aminophenol, p-aminophenol, 5-amino-2-oxytoluene, 2-amino-3-oxy-toluene, 2-oxy-3-amino-1,4-dimethyl-benzene, etc.

Most useful primary aromatic amine type color developing agent includes N,N'-dialkyl-p-phenylenediamine compound, wherein the alkyl group and the phenyl group may be substituted with any substituent. Of these, examples of particularly useful compounds may include N,N'-dimethyl-p-phenylenediamine hydrochloride, N-methyl-p-phenylenediamine hydrochloride, N,N'-dimethyl-p-phenylenediamine hydrochloride, 2-amino-5-(N-ethyl-N-dodecylamino)-toluene, N-ethyl-N-β-methanesulfonamidoethyl-3-methyl-4-aminoaniline sulfate, N-ethyl-N-β-hydroxyethylaminoaniline, 4-amino-3-methyl-N,N'-diethylaniline, 4-amino-N-(2-methoxyethyl)-N-ethyl-3-methylaniline-p-toluene sulfonate, etc.

In addition to the above primary aromatic amine type color developing agent, the color developing agent

used in the processing according to this invention may also optionally contain various components usually added to a color developing agent, for example, alkali agents such as sodium hydroxide, sodium carbonate and potassium carbonate, alkali metal sulfites, alkali metal bisulfites, alkali metal thiocyanates, alkali metal halides, benzyl alcohol, water softeners, thickening agents, etc. This color developing solution may have usually the pH of 7 or more, most usually about 10 to 13.

In this invention, after color developing processing, processing by use of a processing solution having fixing ability is carried out. When the processing solution having fixing ability is a fixing solution, a bleaching is carried out beforehand. As a bleaching agent used in the bleaching step, there may be used a metal complex salt of an organic acid. The metal complex salt has an action to oxidize a metal silver formed by development to allow it to revert to silver halide, and, at the same time, color-develop a non-image portion of a coupler. It has the structure in which an ion of a metal such as iron, cobalt, copper, etc. is coordinated with an organic acid such as an aminopolycarboxylic acid or oxalic acid, citric acid, etc. The organic acid most preferably used for the formation of the metal complex salt of such an organic acid may include polycarboxylic acid or aminopolycarboxylic acid. The polycarboxylic acid or aminopolycarboxylic acid may be in the form of an alkali metal salt, an ammonium salt or a water soluble amine salt.

Typical examples of these may include the following:

- (1) Ethylenediaminetetraacetic acid
- (2) Nitrilotriacetic acid
- (3) Iminodiacetic acid
- (4) Disodium ethylenediaminetetraacetate
- (5) Tetra(trimethylammonium) ethylenediaminetetraacetate
- (6) Tetrasodium ethylenediaminetetraacetate
- (7) Sodium nitrilotriacetate

A bleaching solution to be used may contain as the bleaching agent the above metal complex salt of the organic acid, and also contain various additives. Preferably, the additive to be contained may include, in particular, re-halogenating agents such as an alkali halide and an ammonium halide, for example, potassium bromide, sodium bromide, sodium chloride, ammonium bromide, etc., a metal salt and a chelating agent. Also, there may be optionally added those which are known to be usually added to a bleaching solution, including pH buffering agents such as borate, oxalate, acetate, carbonate and phosphate, alkylamines, polyethyleneoxides, etc.

Further, the fixing solution and bleach-fixing solution may contain a pH buffering agent including sulfites such as ammonium sulfite, potassium sulfite, ammonium bisulfite, potassium bisulfite, sodium bisulfite, ammonium metabisulfite, potassium metabisulfite and sodium metabisulfite, and boric acid, borax, sodium hydroxide, potassium hydroxide, sodium carbonate, potassium carbonate, sodium bisulfite, sodium bicarbonate, potassium bicarbonate, acetic acid, sodium acetate, ammonium hydroxide, etc., which may be added singularly or in combination of two or more.

When the processing of this invention is carried out while replenishing a bleach-fixing replenishing agent in a bleach-fixing solution (or bath), the bleach-fixing solution (or bath) may contain a thiosulfate, a thiocyanate or a sulfite, etc., or these salts may be contained in a bleach-fixing replenishing solution which is replenished to the processing bath.

In this invention, if desired, blowing of air or blowing of oxygen may be carried out in the bleach-fixing bath and in a storage tank for the bleach-fixing replenishing solution in order to enhance the activity in the bleach-fixing solution, or a suitable oxidizing agent including, for example, hydrogen peroxide, bromate, persulfate, etc. may be added.

According to the light-sensitive silver halide photographic material of this invention, it has excellent color reproducibility, has been remarkably improved in the fastness to light of a magenta dye image, and also can prevent the generation of color fog.

This invention will be described specifically by referring to the following Examples, by which, however, embodiments of this invention are not limited.

15

### EXAMPLE 1

Various coupler dispersions were prepared with the formulation as shown in Table 1 and according to the method shown below, and the resulting dispersions were mixed into 500 g each of green-sensitive silver chlorobromide emulsion. The mixture were then applied to supports made of polyethylene-coated paper to obtain Samples 1 to 28.

25

### (PREPARATION OF COUPLER DISPERSIONS)

Forty grams (40 g) of magenta coupler shown in Table 1, the anti-color-fading agent shown in Table 1 (50 mole % based on the coupler) and the hydroquinone derivative shown in Table 1 were dissolved in a mixed solvent comprising 40 ml of dioctylphthalate and 100 ml of ethyl acetate, and the solution obtained was added to 300 ml of a 5% aqueous gelatin solution containing sodium dodecylbenzenesulfonate, followed by dispersion by use of an ultrasonic homogenizer to give each of 35 the coupler dispersion.

Samples thus obtained were subjected to wedge exposure according to a conventional method, followed by carrying out the following processing.

40

#### Standard processing steps (Processing temperature and processing time):

|                        |           |                |
|------------------------|-----------|----------------|
| [1] Color developing   | 38° C.    | 3 min. 30 sec. |
| [2] Bleach-fixing      | 33° C.    | 1 min. 30 sec. |
| [3] Washing with water | 25-30° C. | 3 min.         |
| [4] Drying             | 75-80° C. | about 2 min.   |

45

$$\text{Retention} = \frac{D}{D_0} \times 100 (\%)$$

(D = density after color-fading)

Minimum reflection density of each of the samples thus processes was measured to evaluate the characteristics for "color fog".

TABLE 1

| Sample No. | Magenta coupler       | Anti-color-fading agent |         | Hydroquinone derivative |         | Fastness to light (%) | Color fog (Dmin) | Comparative example |
|------------|-----------------------|-------------------------|---------|-------------------------|---------|-----------------------|------------------|---------------------|
|            |                       | Kind                    | Eox (v) | Kind                    | Amount* |                       |                  |                     |
| 1          | Comparative example-1 | —                       | —       | HQ-4                    | 0.10    | 53                    | 0.03             | Comparative example |
| 2          | Comparative example-1 | —                       | —       | "                       | 0.50    | 55                    | "                | "                   |
| 3          | Comparative example-1 | AO-6                    | 1.13    | "                       | "       | 67                    | "                | "                   |
| 4          | 44                    | —                       | —       | "                       | 0.10    | 22                    | "                | "                   |
| 5          | "                     | —                       | —       | "                       | 0.50    | 19                    | "                | "                   |
| 6          | "                     | AO-6                    | 1.13    | —                       | —       | 66                    | 0.05             | "                   |
| 7          | "                     | "                       | "       | HQ-4                    | 0.01    | 68                    | 0.03             | Present invention   |
| 8          | "                     | "                       | "       | "                       | 0.04    | 67                    | "                | "                   |
| 9          | "                     | "                       | "       | "                       | 0.10    | 62                    | "                | "                   |
| 10         | "                     | "                       | "       | "                       | 0.20    | 45                    | "                | Comparative example |
| 11         | "                     | "                       | "       | "                       | 0.50    | 32                    | 0.02             | "                   |
| 12         | "                     | AO-1                    | 1.01    | "                       | 0.04    | 68                    | 0.03             | Present invention   |
| 13         | "                     | AO-4                    | 1.03    | "                       | "       | 66                    | "                | "                   |
| 14         | "                     | AO-13                   | 1.09    | "                       | "       | 67                    | "                | "                   |
| 15         | "                     | AO-10                   | 1.39    | "                       | "       | 68                    | "                | "                   |
| 16         | "                     | AO-23                   | 1.27    | "                       | "       | 69                    | "                | "                   |

### Composition of processing solutions:

| (Color developing solution)                                                                                                                 |         |
|---------------------------------------------------------------------------------------------------------------------------------------------|---------|
| Benzyl alcohol                                                                                                                              | 15 ml   |
| Ethylene glycol                                                                                                                             | 15 ml   |
| Potassium sulfite                                                                                                                           | 2.0 g   |
| Potassium bromide                                                                                                                           | 0.7 g   |
| Sodium chloride                                                                                                                             | 0.2 g   |
| Potassium carbonate                                                                                                                         | 30.0 g  |
| Hydroxylamine sulfate                                                                                                                       | 3.0 g   |
| Polyphosphorous acid (TPPS)                                                                                                                 | 2.5 g   |
| 3-Methyl-4-amino-N-ethyl-N-(ethyl<br>β-methanesulfonamide)-                                                                                 | 5.5 g   |
| aniline sulfate                                                                                                                             |         |
| Brightening agent (a 4,4'-diamino-<br>styrene sulfonic acid derivative)                                                                     | 1.0 g   |
| Potassium hydroxide                                                                                                                         | 2.0 g   |
| Made up to one liter in total amount<br>by adding water, and adjusted<br>to pH 10.20.                                                       |         |
| (Bleach-fixing solution)                                                                                                                    |         |
| Ferric ammonium ethylenediamine-<br>tetraacetate dihydrate                                                                                  | 60 g    |
| Ethylenediaminetetraacetic acid                                                                                                             | 3 g     |
| Ammonium thiosulfate (70% solution)                                                                                                         | 100 ml  |
| Ammonium sulfite (40% solution)                                                                                                             | 27.5 ml |
| Adjusted to pH 7.1 by use of potassium<br>carbonate or glacial acetic acid,<br>and made up to one liter in total<br>amount by adding water. |         |

After the processing, the fastness to light of the magenta dye images obtained was tested according to the method shown below. Results obtained are shown in Table 1.

### (FASTNESS-TO-LIGHT TEST)

The fastness to light was indicated in terms of the retention of the initial density  $D_0=1$  when irradiated with sunlight for 30 days using an underglass weathering stand.

TABLE 1-continued

| Sample No. | Magenta coupler | Anti-color-fading agent |         | Hydroquinone derivative |         | Fastness to light (%) | Color fog (Dmin) |
|------------|-----------------|-------------------------|---------|-------------------------|---------|-----------------------|------------------|
|            |                 | Kind                    | Eox (v) | Kind                    | Amount* |                       |                  |
| 17         | "               | AO-28                   | 1.34    | "                       | "       | 69                    | 0.02             |
| 18         | "               | AO-29                   | 1.10    | "                       | "       | 64                    | 0.03             |
| 19         | "               | CACFA**-1               | 1.72    | "                       | "       | 39                    | "                |
| 20         | "               | CACFA**-2               | 0.82    | "                       | "       | 37                    | "                |
| 21         | 59              | AO-6                    | 1.13    | "                       | "       | 68                    | "                |
| 22         | 99              | "                       | "       | "                       | "       | 68                    | "                |
| 23         | 130             | "                       | "       | "                       | "       | 67                    | "                |
| 24         | 5               | "                       | "       | "                       | "       | 66                    | "                |
| 25         | 157             | "                       | "       | "                       | "       | 68                    | "                |
| 26         | 44              | "                       | "       | HQ-3                    | "       | 67                    | "                |
| 27         | "               | "                       | "       | HQ-14                   | "       | 66                    | "                |
| 28         | "               | "                       | "       | HQ-16                   | "       | 68                    | "                |

\*Amount of hydroquinone derivative is expressed by molar amount based on magenta coupler

#### \*\*Comparative anti-color-fading agent



As will be seen from the results shown in Table 1, comparing Sample 1 with Sample 2, the hydroquinone derivative (HQ-4) has improved the fastness to light of the magenta dye with respect to comparative magenta coupler 1 as conventionally known, and, in Sample 3 to which the anti-color-fading agent (AO-6) was added, the fastness to light has been much better improved. However, in Samples 1 to 3 employing comparative magenta coupler 1, the magenta dyes obtained, which have a secondary absorption in the spectral absorption characteristics as mentioned above, show undesirable color reproducibility.

On the other hand, comparing Sample 4 with Sample 5, results are different from the case where the above comparative magenta coupler 1, i.e., 3-anilino-5-pyrazolone type magenta coupler was added, and there can not be seen any improvement at all in the fastness to light of the magenta dye obtained from exemplary magenta coupler 44 when the hydroquinone derivative was used in such an increased amount as described in Japanese Unexamined Patent Publication No. 125732/1984, and

20 moreover the fastness to light has been deteriorated on the contrary.

Among Samples 6 to 11 employing the anti-color-fading agent according to this invention, Samples 7, 8 and 9 in which the hydroquinone derivatives are within the scope of this invention show highest values. Although high fastness to light is shown also in Sample 6, color fog is too high for the product to be practically usable.

It is also clear from Samples 12 to 20 wherein the oxidation potential of the anti-color-fading agent was varied, that high fastness to light can not be obtained even when the anti-color-fading agent whose oxidation potential  $E_{ox}$  does not fall in the scope of  $0.95 \leq E_{ox} \leq 1.50$  (V) was combined.

35 In Samples 21 to 28, good fastness to light was achieved in the same manner as above, when the kinds of magenta couplers and hydroquinone derivatives were varied.

The spectral absorption characteristics of the magenta dyes obtained in Samples 4 to 28 showed low secondary absorption to give desirable color reproducibility.

45 Thus, as to the fastness to light of the magenta dye image obtained from the magenta coupler having particular structure, the effect obtainable from the combination with the anti-color-fading agent used in the particular range becomes remarkably cooperative only when the hydroquinone derivative is used in the range of an amount greatly smaller than that conventionally used, thereby achieving dramatical improvement in the 50 fastness to light. This was found to be a fact that could not be expected from conventional techniques.

### EXAMPLE 2

55 A support made of polyethylene-coated paper was provided with the following respective layers successively from the side of the support to produce a multi-color silver halide color photographic material.

First layer: Blue-sensitive silver halide emulsion layer  
 Coated were  $\alpha$ -pivalyl- $\alpha$ -(1-benzyl-2,4-dioxoimidazolidin-3-yl)-2-chloro-5-[ $\gamma$ -(2,4-di-t-amylphenoxy)butylamide]-acetoanilide as a yellow coupler to have a coating weight of 3 mg/dm<sup>2</sup>; a blue-sensitive silver chlorobromide emulsion, 8 mg/dm<sup>2</sup> calculated in terms of silver; S-6, 3 mg/dm<sup>2</sup>; and gelatin, 16 mg/dm<sup>2</sup>.

65 Second layer: Intermediate layer

Coated were hydroquinone derivative (HQ-4) to have a coating weight of 0.45 mg/dm<sup>2</sup>; and gelatin, 4 mg/dm<sup>2</sup>.

Third layer: Green-sensitive silver chlorobromide emulsion layer

Coated were comparative magenta coupler 2 to have a coating weight of 4 mg/dm<sup>2</sup>; the above comparative anti-color-fading agent 1 in amount of 50 mole % based on the magenta coupler; the above exemplary hydroquinone derivative (HQ-3) in the amount shown in Table 2; a green-sensitive silver chlorobromide emulsion to have a coating weight of 4 mg/dm<sup>2</sup> calculated in terms of silver; S-13, 4 mg/dm<sup>2</sup>; and gelatin, 16 mg/dm<sup>2</sup>. 5

Fourth layer: Intermediate layer

Coated were ultraviolet absorbent (UV-1) to have a coating weight of 3 mg/dm<sup>2</sup>; ultraviolet absorbent (UV-2), 3 mg/dm<sup>2</sup>; S-2; 4 mg/dm<sup>2</sup>; hydroquinone derivative (HQ-4), 0.45 mg/dm<sup>2</sup>; and gelatin, 14 mg/dm<sup>2</sup>. 10

Fifth layer: Red-sensitive silver chlorobromide emulsion layer

Coated were 2,4-dichloro-3-methyl-6-[ $\alpha$ -(2,4-di-t-amyloxy)butylamide]-phenol as a cyan coupler to have a coating weight of 1 mg/dm<sup>2</sup>; 2-(2,3,4,5,6-penta-20 fluorophenyl)acylamino-4-chloro-5-[ $\alpha$ -(2,4-di-t-amyloxy)pentylamide], 3 mg/dm<sup>2</sup>; S-2, 2 mg/dm<sup>2</sup>; a red-sensitive silver chlorobromide emulsion, 3 mg/dm<sup>2</sup> calculated in terms of silver; and gelatin, 14 mg/dm<sup>2</sup>. 25

Sixth layer: Intermediate layer

Coated were ultraviolet absorbent (UV-1) to have a coating weight of 2 mg/dm<sup>2</sup>; ultraviolet absorbent (UV-2), 2 mg/dm<sup>2</sup>; S-2, 2 mg/dm<sup>2</sup>; and gelatin 6 mg/dm<sup>2</sup>. 30

Seventh layer: Protective layer

Coated was gelatin to have a coating weight of 9 mg/dm<sup>2</sup>. 35

A sample thus obtained were designated as Sample 1.

Subsequently, Samples 2 to 7 were produced in the same manner as in Sample 1 except that the combination 35 for the magenta coupler, the anti-color-fading agent, the hydroquinone derivative, the high-boiling solvent and the coated silver weight was made as shown in Table 2. However, the coating weight for the magenta coupler and the anti-color-fading agent each was made equimo- 40 lar to Sample 1.

On these samples, optical wedge exposure was carried out using a sensitometer (KS-7 Type produced by Konishiroku Photo Industry Co., Ltd.), followed by the same processing as in Example 1.

(UV-1):



(UV-2):



Comparative magenta coupler 2:



Comparative magenta coupler 3:



TABLE 2

| Sample No. | Formulation of third layer                 |                       |                         |         |                         |         |                              |                       |                  |
|------------|--------------------------------------------|-----------------------|-------------------------|---------|-------------------------|---------|------------------------------|-----------------------|------------------|
|            | Coated silver weight (mg/dm <sup>2</sup> ) | Magenta coupler       | Anti-color-fading agent |         | Hydroquinone derivative |         | High boiling organic solvent | Fastness to light (%) | Color fog (Dmin) |
|            |                                            |                       | Kind                    | Eox (V) | Kind                    | Amount* |                              |                       |                  |
| 1          | 4.0                                        | Comparative example-2 | **                      | 1.72    | HQ-3                    | 0.20    | S-13                         | 77                    | 0.04 X           |
| 2          | "                                          | Comparative example-3 | CACFA-1                 | 0.82    | HQ-4                    | 0.10    | DBP                          | 80                    | " "              |
| 3          | 2.0                                        | 44                    | AO-6                    | 1.13    | "                       | 0.20    | S-2                          | 53                    | " "              |
| 4          | "                                          | "                     | "                       | "       | "                       | 0.03    | "                            | 79                    | " Y              |
| 5          | "                                          | 1                     | "                       | "       | "                       | "       | "                            | 81                    | " "              |
| 6          | "                                          | 172                   | "                       | "       | "                       | "       | S-6                          | 80                    | " "              |
| 7          | "                                          | 54                    | "                       | "       | "                       | "       | TCP                          | 77                    | " "              |

In Table, DBP represents dibutyl phthalate, and TCP represents tricresyl phosphate.

\*Amount of hydroquinone derivative is expressed by molar amount based on magenta coupler.

\*\*Comparative anti-color-fading agent.

X: Comparative example

Y: Present invention

Samples thus obtained were tested for the fastness to 65 light and the color fog characteristics in the same manner as in Example 1. Results obtained are shown in Table 2.

It is seen from the results in Table 2 that the same results as in Example 1 are obtained also in the multi-color light-sensitive silver halide color photographic material. According to evaluation on the color repro-

ducibility in actual print, Samples 3 to 7 employing magenta couplers according to this invention showed better reproducibility particularly in violet than Samples 1 and 2 employing comparative magenta couplers.

In other words, it is clear that good color reproducibility and high fastness to light have been achieved in Samples 4 to 7 which are in accordance with this invention.

What is claimed is:

1. A light-sensitive silver halide photographic material comprising a support and provided thereon at least one silver halide emulsion layer, wherein at least one layer of said silver halide emulsion layer contains (i) a magenta color forming coupler represented by general formula (I),



(I)

wherein Z represents a group of non-metallic atoms necessary to complete a nitrogen-containing heterocyclic ring which may have a substituent; X represents a hydrogen atom or a substituent capable of being split off upon reaction with an oxidation product of a color developing agent; and R represents a hydrogen atom or a substituent; (ii) at least one anti-color-fading agent having an oxidation potential (E<sub>ox</sub>) of 0.95 (V)  $\leq$  E<sub>ox</sub>  $\leq$  1.50 (V); and (iii) a hydroquinone derivative in an amount ranging from  $1 \times 10^{-3}$  to  $1 \times 10^{-1}$  mole per 1 mole of said magenta color forming coupler represented by formula (I).

2. The light-sensitive silver halide photographic material of claim 1, wherein said substituent for R in formula (I) is selected from the group consisting of a halogen atom, an alkyl group, a cycloalkyl group, an alkenyl group, an cycloalkyl group, an alkynyl group, an aryl group, a heterocyclic group, an acyl group, a sulfonyl group, a sulfinyl group, a phosphonyl group, a carbamoyl group, a sulfamoyl group, a cyano group, a spiro compound residual group, a bridged hydrocarbon compound residual group, an alkoxy group, an aryloxy group, a heterocyclic oxy group, a siloxy group, an acyloxy group, a carbamoyloxy group, an amino group, an acylamino group, a sulfonamide group, an imide group, a ureido group, a sulfamoylamino group, an alkoxycarbonylamino group, an aryloxycarbonylamino group, an alkoxy carbonyl group, an aryloxycarbonyl group, an alkylthio group, an arylthio group and a heterocyclic thio group.

3. The light-sensitive silver halide photographic material of claim 1, wherein X in formula (I) is selected from the group consisting of a halogen atom and an organic group having a carbon atom, an oxygen atom, a sulfur atom, or a nitrogen atom through which said organic group is connected with the remainder of the compound.

4. The light-sensitive silver halide photographic material of claim 1, wherein X in formula (I) is selected from the group consisting of a halogen atom, an alkoxy group, an aryloxy group, a heterocyclic oxy group, an acyloxy group, a sulfonyloxy group, an alkoxycarbonyloxy group, an aryloxycarbonyloxy group, an alkylxaryloxy group, an alkoxyoxalyloxy group, an alkylthio group, an arylthio group, a heterocyclicthio

group, an alkyloxythiocarbonylthio group, a group represented by the formula



10 (wherein R<sup>4'</sup> and R<sup>5'</sup> independently represent a hydrogen atom, an alkyl group, an aryl group, a heterocyclic group, a sulfamoyl group, a carbamoyl group, an acyl group, a sulfonyl group, an aryloxycarbonyl group, and an alkoxy carbonyl group provided that R<sup>4'</sup> and R<sup>5'</sup> are not simultaneously hydrogen atoms and R<sup>4'</sup> and R<sup>5'</sup> may combine with each other to form a nitrogen-containing heterocyclic group),

20 a carboxyl group, a hydroxymethyl group, a triphenylmethyl group and a group represented by the following formula:



25 (wherein R<sup>1</sup> is defined to be the same as R, Z' is the same as defined for Z, and R<sup>2</sup> and R<sup>3</sup> are independently selected from the group consisting of a hydrogen atom, an aryl group, an alkyl group and a heterocyclic group.)

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720



(XII)

5

wherein, R<sup>1</sup> and R<sup>2</sup> are independently selected from the group consisting of an alkyl group, an aryl group, an alkenyl group and a cycloalkyl group; and a compound of general formula (XIII) or a precursor thereof:



(XIII)

wherein, R<sup>3</sup> and R<sup>4</sup> are independently selected from an alkyl group having 1 to 5 carbon atoms, R<sup>5</sup> is selected from the group consisting of an alkyl group, an aryl group, an alkenyl group, a cycloalkyl group and a group represented by a formula



35

Q is selected from the group consisting of

(a) —COXR<sup>6</sup> group wherein X is an oxygen atom or

a



group wherein R<sup>7</sup> is selected from the group consisting of a hydrogen atom, an alkyl group or an aryl group, R<sup>6</sup> is selected from the group consisting of a hydrogen atom, an alkyl group, an alkenyl group, a cycloalkyl group and an aryl group,

(b) a —OY group wherein Y is R<sup>6</sup> or a —COR<sup>6</sup> group,

(c)

(XII)

10

10

15

20

25

30

35

40

45

50

55

60



group wherein R<sup>8</sup> is a selected from the group consisting of a hydrogen atom, an alkyl group, an aryl group and a —COR<sup>6</sup> group,

(d) a—P(O)(OR<sup>6</sup>)<sub>2</sub> ((O)l R<sup>9</sup>) group wherein R<sup>9</sup> is defined to have the same meaning as R<sup>6</sup> and l is 0 or 1 and

(e) a cyano group, n is an integer of 1 to 20 and k is an integer of 1 or 2.

15 10. The light-sensitive silver halide photographic material of claim 1, wherein said anti-color-fading agent has an oxidation potential (Eox) of 1.00 (V)  $\leq$  Eox  $\leq$  1.45 (V).20 11. The light-sensitive silver halide photographic material of claim 10, wherein said anti-color-fading agent has an oxidation potential (Eox) of 1.00 (V)  $\leq$  Eox  $\leq$  1.40 (V).

25 12. The light-sensitive silver halide photographic material of claim 1, wherein said hydroquinone derivative is selected from the group consisting of a compound represented by general formula (XII') and a precursor thereof;



wherein, R<sup>10</sup> and R<sup>11</sup> independently represent a hydrogen atom or an alkyl group having 1 to 5 carbon atoms and R<sup>6</sup> has the same meaning as defined in formula (XIII), provided that R<sup>10</sup> and R<sup>11</sup> are not simultaneously hydrogen atoms.

13. The light-sensitive silver halide photographic material of claim 1, wherein said hydroquinone derivative is selected from the group consisting of a compound represented by general formula (XIII') and a precursor thereof;



wherein R<sup>3</sup>, R<sup>4</sup>, R<sup>6</sup> and n have the same definition as in formula (XIII).

\* \* \* \* \*

65

60

UNITED STATES PATENT AND TRADEMARK OFFICE  
CERTIFICATE OF CORRECTION

PATENT NO. : 5,006,454

DATED : April 9, 1991

INVENTOR(S) : Masao Sasaki, et al.

It is certified that error appears in the above-identified patent and that said Letters Patent is hereby corrected as shown below:

Claim 2, column 141, line 40, before "cycloalkyl" change "an" to --a--.

Claim 4, column 142, line 14, before "and" delete ",,.

Claim 4, column 142, line 15, after "group" insert --,--.

Claim 4, column 142, line 32, change "R<sup>1</sup>" to --R<sup>1</sup>'--.

Claim 7, column 142, line 53, change "hydroquinine" to --hydroquinone--.

Claim 9, column 143, line 59, after "(c)" insert --a--.

Claim 9, column 144, line 4, change "a-N<sup>R<sup>7</sup><sub>R<sup>8</sup></sub>" to -- -N<sup>R<sup>7</sup><sub>R<sup>8</sup></sub> --.

Claim 9, column 144, line 7, after "is" delete "a".

Signed and Sealed this  
Eighteenth Day of May, 1993

Attest:



MICHAEL K. KIRK

Attesting Officer

Acting Commissioner of Patents and Trademarks